



US011155764B2

(12) **United States Patent**  
**Yang et al.**

(10) **Patent No.:** **US 11,155,764 B2**  
(b5) **Date of Patent:** **Oct. 26, 2021**

(54) **LUBRICANTS FOR USE IN BOOSTED ENGINES**

- (71) Applicant: **Afton Chemical Corporation**, Richmond, VA (US)
- (72) Inventors: **Kongsheng Yang**, Glen Allen, VA (US); **Kristin Fletcher**, Midlothian, VA (US); **William Y. Lam**, Glen Allen, VA (US); **Jeremy Styer**, Glen Allen, VA (US)
- (73) Assignee: **AFTON CHEMICAL CORPORATION**, Richmond, VA (US)
- (\*) Notice: Subject to any disclaimer, the term of this patent is extended or adjusted under 35 U.S.C. 154(b) by 270 days.

(21) Appl. No.: **15/409,514**

(22) Filed: **Jan. 18, 2017**

(65) **Prior Publication Data**

US 2017/0321145 A1 Nov. 9, 2017

**Related U.S. Application Data**

(63) Continuation-in-part of application No. 15/147,375, filed on May 5, 2016, now Pat. No. 10,421,922.

(51) **Int. Cl.**

**C10M 135/10** (2006.01)  
**C10M 171/00** (2006.01)  
**C10M 163/00** (2006.01)  
**C10M 129/50** (2006.01)  
**C10M 139/00** (2006.01)  
**C10N 10/04** (2006.01)  
**C10N 10/12** (2006.01)  
**C10N 30/04** (2006.01)  
**C10N 30/08** (2006.01)  
**C10N 30/10** (2006.01)  
**C10N 30/00** (2006.01)  
**C10N 40/25** (2006.01)  
**C10N 60/14** (2006.01)

(52) **U.S. Cl.**

CPC ..... **C10M 135/10** (2013.01); **C10M 129/50** (2013.01); **C10M 139/00** (2013.01); **C10M 163/00** (2013.01); **C10M 171/00** (2013.01); **C10M 2203/1025** (2013.01); **C10M 2205/0285** (2013.01); **C10M 2207/028** (2013.01); **C10M 2207/262** (2013.01); **C10M 2219/046** (2013.01); **C10M 2227/00** (2013.01); **C10N 2010/04** (2013.01); **C10N 2010/12** (2013.01); **C10N 2030/04** (2013.01); **C10N 2030/10** (2013.01); **C10N 2030/40** (2020.05); **C10N 2030/52** (2020.05); **C10N 2040/25** (2013.01); **C10N 2040/255** (2020.05); **C10N 2060/14** (2013.01)

(58) **Field of Classification Search**

CPC . C10M 135/10; C10M 129/50; C10M 139/00  
See application file for complete search history.

(56)

**References Cited**

U.S. PATENT DOCUMENTS

|             |         |                 |
|-------------|---------|-----------------|
| 3,185,647 A | 5/1965  | Anderson et al. |
| 3,189,544 A | 6/1965  | Hyman et al.    |
| 3,256,185 A | 6/1966  | Le Suer         |
| 3,278,550 A | 10/1966 | Norman et al.   |
| 3,312,619 A | 4/1967  | Dale            |
| 3,366,569 A | 1/1968  | Norman et al.   |
| 3,390,086 A | 6/1968  | Rosemary et al. |
| 3,403,102 A | 9/1968  | Le Suer         |
| 3,458,530 A | 7/1969  | Siegel et al.   |
| 3,470,098 A | 9/1969  | O'Halloran      |
| 3,502,677 A | 3/1970  | Sner            |
| 3,519,564 A | 7/1970  | Vogel           |
| 3,546,243 A | 12/1970 | Coupland        |
| 3,573,205 A | 3/1971  | Lowe et al.     |
| 3,634,515 A | 1/1972  | Piasek et al.   |
| 3,649,229 A | 3/1972  | Otto            |

(Continued)

FOREIGN PATENT DOCUMENTS

|    |           |         |
|----|-----------|---------|
| CN | 1453348 A | 11/2003 |
| CN | 1510115 A | 7/2004  |

(Continued)

OTHER PUBLICATIONS

Final Office Action; dated May 24, 2017 for U.S. Appl. No. 15/147,330.

International Search Report and Written Opinion; dated Jun. 9, 2017 for PCT Application No. PCT/US2017/023622.

International Search Report with Written Opinion; dated Jun. 21, 2017 for PCT Application No. PCT/US2017/015279.

International Search Report and Written Opinion; dated Oct. 6, 2016 for PCT Application No. PCT/US2016/042332.

(Continued)

*Primary Examiner* — Ellen M McAvoy

(74) *Attorney, Agent, or Firm* — Mendelsohn Dunleavy, P.C.

(57) **ABSTRACT**

A lubricating oil composition and method of operating a boosted internal combustion engine. The lubricating oil composition includes greater than 50 wt. % of a base oil of lubricating viscosity, calcium, nitrogen, molybdenum and boron. The weight ratio of Ca:N (ppm/ppm) in the lubricating oil composition is greater than 1.3 to less than 3.0, the weight ratio of Ca:Mo (ppm/ppm) in the lubricating oil composition is greater than 6.7 to less than 56.3, and the weight ratio of Ca:B (ppm/ppm) in the lubricating oil composition is greater than 5.0 to less than 9.8. The lubricating oil composition does not contain added magnesium from a magnesium-containing detergent. The lubricating oil composition is resistant to deposit formation in the boosted internal combustion engine, as shown by its ability to ensure a TCO Temperature Increase of less than 9.0% as measured using the 2015 version of the General Motors dexos1® Turbocharger Coking Test.

| (56)                  | References Cited |                     |                  |         |                               |  |
|-----------------------|------------------|---------------------|------------------|---------|-------------------------------|--|
| U.S. PATENT DOCUMENTS |                  |                     |                  |         |                               |  |
| 3,708,522 A           | 1/1973           | LeSuer              | 7,645,726 B2     | 1/2010  | Loper                         |  |
| 3,718,663 A           | 2/1973           | Lee et al.          | 7,727,943 B2     | 6/2010  | Brown et al.                  |  |
| 3,749,695 A           | 7/1973           | De Vries            | 7,732,390 B2     | 6/2010  | Kadkhodayan et al.            |  |
| 3,859,318 A           | 1/1975           | Le Suer             | 7,776,800 B2     | 8/2010  | Lam et al.                    |  |
| 3,865,740 A           | 2/1975           | Goldschmidt         | 7,820,599 B2     | 10/2010 | Kasai                         |  |
| 3,865,813 A           | 2/1975           | Gergel              | 7,820,602 B2     | 10/2010 | Ravichandran et al.           |  |
| 3,954,639 A           | 5/1976           | Liston              | 7,897,696 B2     | 3/2011  | Huang et al.                  |  |
| 4,152,499 A           | 5/1979           | Boerzel et al.      | 7,906,469 B2     | 3/2011  | Arrowsmith et al.             |  |
| 4,234,435 A           | 11/1980          | Meinhardt et al.    | 8,048,831 B2     | 11/2011 | Loper                         |  |
| 4,259,194 A           | 3/1981           | DeVries et al.      | 8,163,681 B2     | 4/2012  | Bardasz et al.                |  |
| 4,259,195 A           | 3/1981           | King et al.         | 8,334,243 B2     | 12/2012 | Guevremont et al.             |  |
| 4,261,843 A           | 4/1981           | King et al.         | 8,415,284 B2     | 4/2013  | Duggal                        |  |
| 4,263,152 A           | 4/1981           | King et al.         | 8,586,517 B2     | 11/2013 | Waynick                       |  |
| 4,265,773 A           | 5/1981           | DeVries et al.      | 8,709,988 B2     | 4/2014  | Arrowsmith et al.             |  |
| 4,272,387 A           | 6/1981           | King et al.         | 8,999,905 B2     | 4/2015  | Duggal                        |  |
| 4,283,295 A           | 8/1981           | DeVries et al.      | 9,359,576 B2     | 6/2016  | Yoshida                       |  |
| 4,285,822 A           | 8/1981           | DeVries et al.      | 9,528,074 B2     | 12/2016 | Hogendoorn                    |  |
| 4,379,064 A           | 4/1983           | Cengel et al.       | 10,155,915 B2    | 12/2018 | Tamura                        |  |
| 4,482,464 A           | 11/1984          | Karol et al.        | 10,227,544 B2    | 3/2019  | Kim et al.                    |  |
| 4,521,318 A           | 6/1985           | Karol               | 2002/0019320 A1  | 2/2002  | Nakazato et al.               |  |
| 4,554,086 A           | 11/1985          | Karol et al.        | 2002/0038525 A1  | 4/2002  | Callis et al.                 |  |
| 4,579,675 A           | 4/1986           | Sawicki et al.      | 2002/0058593 A1  | 5/2002  | Bovington et al.              |  |
| 4,612,132 A           | 9/1986           | Wollenberg et al.   | 2002/0151441 A1  | 10/2002 | Srinivasan et al.             |  |
| 4,614,522 A           | 9/1986           | Buckley             | 2004/0176260 A1  | 9/2004  | Shirahama et al.              |  |
| 4,614,603 A           | 9/1986           | Wollenberg          | 2005/0153848 A1  | 7/2005  | Bell et al.                   |  |
| 4,617,137 A           | 10/1986          | Plavac              | 2006/0058200 A1  | 3/2006  | Shaw et al.                   |  |
| 4,617,138 A           | 10/1986          | Wollenberg          | 2006/0084582 A1  | 4/2006  | Wells et al.                  |  |
| 4,636,322 A           | 1/1987           | Nalesnik            | 2006/0116299 A1  | 6/2006  | Arrowsmith et al.             |  |
| 4,645,515 A           | 2/1987           | Wollenberg          | 2006/0116302 A1  | 6/2006  | Deckman et al.                |  |
| 4,647,390 A           | 3/1987           | Buckley, III et al. | 2006/0217271 A1  | 9/2006  | Brown et al.                  |  |
| 4,648,886 A           | 3/1987           | Buckley, III et al. | 2006/0223718 A1  | 10/2006 | Bastien et al.                |  |
| 4,648,980 A           | 3/1987           | Erdman              | 2006/0276352 A1  | 12/2006 | Vinci                         |  |
| 4,652,387 A           | 3/1987           | Andress, Jr. et al. | 2007/0119390 A1  | 5/2007  | Herrmann et al.               |  |
| 4,663,062 A           | 5/1987           | Wollenberg          | 2007/0132274 A1  | 6/2007  | Lam et al.                    |  |
| 4,663,064 A           | 5/1987           | Nalesnik et al.     | 2008/009426 A1   | 1/2008  | Iyer et al.                   |  |
| 4,666,459 A           | 5/1987           | Wollenberg          | 2008/0110797 A1  | 5/2008  | Fyfe et al.                   |  |
| 4,666,460 A           | 5/1987           | Wollenberg          | 2008/0128184 A1  | 6/2008  | Loper et al.                  |  |
| 4,668,246 A           | 5/1987           | Wollenberg          | 2008/0194440 A1  | 8/2008  | Ravichandran et al.           |  |
| 4,670,170 A           | 6/1987           | Wollenberg          | 2008/0223330 A1  | 9/2008  | Lam et al.                    |  |
| 4,699,724 A           | 10/1987          | Nalesnik et al.     | 2008/0248981 A1  | 10/2008 | Matsui et al.                 |  |
| 4,713,189 A           | 12/1987          | Nalesnik et al.     | 2008/0280796 A1  | 11/2008 | Guinther et al.               |  |
| 4,713,191 A           | 12/1987          | Nalesnik            | 2008/0318817 A1  | 12/2008 | Yagishita                     |  |
| 4,857,214 A           | 8/1989           | Papay et al.        | 2009/0082233 A1  | 3/2009  | Kasai                         |  |
| 4,948,386 A           | 8/1990           | Sung et al.         | 2009/0192063 A1  | 7/2009  | Gray et al.                   |  |
| 4,954,272 A           | 9/1990           | Jao et al.          | 2009/0318318 A1  | 12/2009 | Mathur et al.                 |  |
| 4,963,275 A           | 10/1990          | Gutierrez et al.    | 2010/0035774 A1  | 2/2010  | Growcott                      |  |
| 4,963,278 A           | 10/1990          | Blain et al.        | 2011/0077181 A1  | 3/2011  | Yagishita                     |  |
| 4,971,598 A           | 11/1990          | Andress et al.      | 2011/0239972 A1  | 10/2011 | Kamano et al.                 |  |
| 4,971,711 A           | 11/1990          | Lundberg et al.     | 2011/0245120 A1  | 10/2011 | Bertram et al.                |  |
| 4,973,412 A           | 11/1990          | Migdal et al.       | 2012/0202723 A1  | 8/2012  | Abbey et al.                  |  |
| 4,981,492 A           | 1/1991           | Blain et al.        | 2013/0030226 A1  | 1/2013  | Teshima et al.                |  |
| 5,026,495 A           | 6/1991           | Emert et al.        | 2014/0106999 A1  | 4/2014  | Nelson et al.                 |  |
| 5,030,249 A           | 7/1991           | Herbstman           | 2014/0274840 A1  | 9/2014  | Esche et al.                  |  |
| 5,039,307 A           | 8/1991           | Herbstman et al.    | 2015/0034047 A1  | 2/2015  | Yaguchi et al.                |  |
| 5,137,647 A           | 8/1992           | Karol               | 2015/0133352 A1  | 5/2015  | Esche et al.                  |  |
| 5,204,012 A           | 4/1993           | Schaffhausen        | 2015/0175924 A1  | 6/2015  | Dance et al.                  |  |
| 5,241,003 A           | 8/1993           | Degonia et al.      | 2015/0307802 A1  | 10/2015 | Ritchie et al.                |  |
| 5,334,321 A           | 8/1994           | Harrison et al.     | 2015/0322367 A1* | 11/2015 | Patel ..... C10M 163/00       |  |
| 5,498,355 A           | 3/1996           | Perozzi et al.      |                  |         | 508/186                       |  |
| 5,650,381 A           | 7/1997           | Gatto et al.        | 2015/0322368 A1* | 11/2015 | Patel ..... C10M 163/00       |  |
| 5,658,862 A           | 8/1997           | Vrahopoulos         |                  |         | 508/192                       |  |
| 5,739,355 A           | 4/1998           | Gateau et al.       | 2015/0322369 A1* | 11/2015 | Patel ..... C10M 163/00       |  |
| 5,804,537 A           | 9/1998           | Boffa et al.        |                  |         | 508/162                       |  |
| 5,883,057 A           | 3/1999           | Roell, Jr. et al.   | 2016/0116299 A1  | 4/2016  | Kim et al.                    |  |
| 6,004,910 A           | 12/1999          | Bloch et al.        | 2016/0230114 A1* | 8/2016  | Aoki ..... C10M 169/04        |  |
| 6,034,040 A           | 3/2000           | Ozbalik et al.      | 2016/0230115 A1* | 8/2016  | Mosier ..... C10M 169/04      |  |
| 6,140,282 A           | 10/2000          | Cartwright et al.   | 2016/0230116 A1* | 8/2016  | Mosier ..... C10M 163/00      |  |
| RE37,363 E            | 9/2001           | Gatto et al.        | 2016/0304802 A1  | 10/2016 | Tamura et al.                 |  |
| 6,300,291 B1          | 10/2001          | Hartley et al.      | 2016/0326453 A1* | 11/2016 | Galic Raguz ..... C10M 163/00 |  |
| 6,569,818 B2          | 5/2003           | Nakazato et al.     | 2017/0015929 A1* | 1/2017  | Fletcher ..... C10M 169/04    |  |
| 6,723,685 B2          | 4/2004           | Hartley et al.      | 2017/0022441 A1* | 1/2017  | Onodera ..... C10M 141/12     |  |
| RE38,929 E            | 1/2006           | Gatto et al.        | 2017/0130158 A1  | 5/2017  | Tamura                        |  |
| 7,214,649 B2          | 5/2007           | Loper et al.        | 2017/0158982 A1* | 6/2017  | Tamura ..... C10M 135/18      |  |
| RE40,595 E            | 12/2008          | Gatto et al.        | 2017/0204348 A1* | 7/2017  | Tamura ..... C10M 165/00      |  |
| 7,550,415 B2          | 6/2009           | Fujitsu et al.      | 2017/0298287 A1  | 10/2017 | Tamura                        |  |
|                       |                  |                     | 2018/0044610 A1* | 2/2018  | Mayhew ..... C10M 169/048     |  |
|                       |                  |                     | 2018/0087001 A1* | 3/2018  | Mosier ..... C10M 133/56      |  |

(56)

## References Cited

## U.S. PATENT DOCUMENTS

2019/0100713 A1\* 4/2019 Utaka ..... C10M 135/10  
 2019/0233758 A1\* 8/2019 Takeshima ..... C10M 101/02

## FOREIGN PATENT DOCUMENTS

CN 1523088 A 8/2004  
 CN 1626632 A 6/2005  
 CN 1746280 A 3/2006  
 CN 1782047 A 6/2006  
 CN 101027380 A 8/2007  
 CN 101184830 A 5/2008  
 CN 101191098 A 6/2008  
 CN 101583702 A 11/2009  
 CN 102676274 A 9/2012  
 CN 102690715 A 9/2012  
 CN 103215108 A 7/2013  
 CN 103642569 A 3/2014  
 CN 104140864 A 11/2014  
 CN 104321416 A 1/2015  
 CN 104342266 A 2/2015  
 CN 104371793 A 2/2015  
 CN 104403721 A 3/2015  
 CN 104560302 A 4/2015  
 CN 105462667 A 4/2016  
 CN 105647616 A 6/2016  
 EP 0317348 A1 5/1989  
 EP 0447916 B1 6/1994  
 EP 0612839 A1 8/1994  
 EP 0839840 A2 5/1998  
 EP 0638632 B1 3/2000  
 EP 1795582 A2 6/2007  
 EP 2371934 A1 10/2011  
 EP 2610333 A1 7/2013  
 EP 2940110 A1 11/2015  
 EP 3101095 A1 12/2016  
 GB 1065595 A1 4/1967  
 GB 2140811 A1 12/1984  
 JP 2005220197 A 8/2005  
 JP 2006117727 A 5/2006  
 JP 2006117729 A 5/2006  
 JP 2006152305 A 6/2006  
 JP 2008274236 A 11/2008  
 JP 2009-501810 A 1/2009  
 JP 2014152301 A1 8/2014  
 JP 2015071788 A 4/2015  
 JP 2016193992 A 11/2016  
 RU 2394069 C2 7/2010  
 SG 106638 A1 10/2004  
 WO WO9731991 A1 9/1997  
 WO WO199947629 A1 9/1999  
 WO 2015023559 A1 2/2015  
 WO 2015042337 A1 3/2015  
 WO 2015042340 A1 3/2015  
 WO 2015042341 A1 3/2015  
 WO WO2015042337 A1 3/2015  
 WO WO2015042340 A1 3/2015  
 WO 2015076417 A1 5/2015  
 WO WO2015114920 A1 8/2015  
 WO WO2015152226 A1 10/2015  
 WO WO2015171981 A1 11/2015  
 WO WO2016043333 A1 3/2016  
 WO WO2016152995 A1 9/2016  
 WO WO2016154167 A1 9/2016  
 WO WO2016159185 A1 10/2016  
 WO WO2017011687 A1 1/2017

## OTHER PUBLICATIONS

European Office Action; dated Jul. 30, 2018 for EP Application No. EP16 741 792.2.  
 European Office Action; dated Aug. 14, 2018 for EP Application No. EP16 741 797.1.  
 Final Office Action; dated Jun. 8, 2018 for U.S. Appl. No. 15/147,330.  
 Non-Final Office Action; dated Jun. 21, 2018 for U.S. Appl. No. 15/409,513.

Non-Final Office Action; dated Oct. 1, 2018 for U.S. Appl. No. 15/147,317.

Non-Final Office Action; dated Oct. 1, 2018 for U.S. Appl. No. 15/147,375.

Non-Final Office Action; dated Oct. 1, 2018 for U.S. Appl. No. 15/147,464.

Final Office Action; dated Jul. 20, 2018 for U.S. Appl. No. 15/147,404.  
 Dahnz, Christoph, et al. "Investigations on pre-ignition in highly supercharged SI engines." *SAE International Journal of Engines* 3.1 (2010): 214-224.

Zahdeh, Akram, et al. "Fundamental approach to investigate pre-ignition in boosted SI engines." *SAE International Journal of Engines* 4.1 (2011): 246-273.

Takeuchi, Kazuo, et al. "Investigation of engine oil effect on abnormal combustion in turbocharged direct injection-spark ignition engines." *SAE International Journal of Fuels and Lubricants* 5.3 (2012): 1017-1024.

Palaveev, Stefan, et al. "Premature Flame Initiation in a Turbocharged DISI Engine-Numerical and Experimental Investigations." *SAE International Journal of Engines* 6.1 (2013): 54-66.

Hirano, Satoshi, et al. Investigation of Engine Oil Effect on Abnormal Combustion in Turbocharged Direct Injection-Spark Ignition Engines (Part 2). No. 2013-01-2569. *SAE Technical Paper*, 2013.  
 Okada, Yoshihiro, et al. "Study of low-speed pre-ignition in boosted spark ignition engine." *SAE International Journal of Engines* 7.2 (2014): 584-594.

Dingle, Simon F., et al. Lubricant induced pre-ignition in an optical SI engine. No. 2014-01-1222. *SAE Technical Paper*, 2014.

Qi, Yunliang, et al. The effect of oil intrusion on super knock in gasoline engine. No. 2014-01-1224. *SAE Technical Paper*, 2014.

Ohtomo, Mitsuaki, et al. "Pre-ignition of gasoline-air mixture triggered by a lubricant oil droplet." *SAE International Journal of Fuels and Lubricants* 7.3 (2014): 673-682.

Fujimoto, Kosuke, et al. "Engine oil development for preventing pre-ignition in turbocharged gasoline engine." *SAE International Journal of Fuels and Lubricants* 7.3 (2014): 869-874.

Moriyoshi, Yasuo, et al. "A Study of Low Speed Preignition Mechanism in Highly Boosted SI Gasoline Engines." *SAE International Journal of Engines* 9.2015-01-1865 (2015).

"Relative Impact of Chemical and Physical Properties of the Oil-Fuel Droplet on Pre-Ignition and Superknock in Turbocharged Gasoline Engines," *SAE 2016 Powertrain Baltimore—Manuscript—Droplet Pre-ignition\_v10*, pp. 1-12.

Ritchie, Andrew, Doyle Boese, and Anne W. Young. "Controlling Low-Speed Pre-Ignition in Modern Automotive Equipment Part 3: Identification of Key Additive Component Types and Other Lubricant Composition Effects on Low-Speed Pre-Ignition." *SAE International Journal of Engines* 9.2016-01-0717 (2016).

Mayer, Mattias, et al. "Influence of Different Oil Properties on Low-Speed Pre-Ignition in Turbocharged Direct Injection Spark Ignition Engines," No. 2016-01-0718. *SAE Technical Paper*, 2016.

Andrews, Arthur, et al. "Investigation of Engine Oil Base Stock Effects on Low Speed Pre-Ignition in a Turbocharged Direct Injection SI Engine," No. 2016-01-9071. *SAE Technical Paper*, 2016.

Fletcher, K. A. et al. "Engine Oil Additive Impacts on Low Speed Preignition," Afton Chemical Corp. *SAE International*, 2016, 7 pages.

EO LSPI IP Discussion Presentation, Feb. 9, 2015, 11 pages.

Update: EO LSPI IP Filing Plan Presentation, Mar. 17, 2015, pp. title-35.

Onodera, Ko, et al. Engine Oil Formulation Technology to Prevent Pre-ignition in Turbocharged Direct Injection Spark Ignition Engines. No. 2015-01-2027. *SAE Technical Paper*, 2015.

Elliott, Ian, et al. Understanding Low Speed Pre-Ignition Phenomena across Turbo-Charged GDI Engines and Impact on Future Engine Oil Design. No. 2015-01-2028. *SAE Technical Paper*, 2015.

Long, Yan, et al. Effect of Oil and Gasoline Properties on Pre-Ignition and Super-Knock in a Thermal Research Engine (TRE) and an Optical Rapid Compression Machine (RCM). No. 2016-01-0720. *SAE Technical Paper*, 2016.

(56)

**References Cited****OTHER PUBLICATIONS**

- Tamura, Kazushi, et al. "Abnormal Combustion Induced by Combustion Chamber Deposits Derived from Engine Oil Additives in a Spark-Ignited Engine." *SAE International Journal of Engines* 8.1 (2015): 200-205.  
Non-Final Office Action; dated Sep. 6, 2017 for U.S. Appl. No. 15/409,513.  
Non-Final Office Action; dated Sep. 6, 2017 for U.S. Appl. No. 15/047,934.  
Non-Final Office Action; dated Nov. 16, 2018 for U.S. Appl. No. 15/147,330.  
International Search Report and Written Opinion; dated Jan. 25, 2018 for PCT Application No. PCT/US2017/060959.  
Jennings, M. A. "Technical Bulletin—TBN in Diesel Engine Oils," Chevron, Feb. 2012 as retrieved on Jan. 16, 2018 from: <http://www.championbrands.com/Tech%20Bulletin%20TBN-Chevron.pdf>, XP055441436.  
International Search Report and Written Opinion; dated Jan. 15, 2018 for PCT Application No. PCT/US2017/060956.  
Ethyl Safety Data Sheet "HiTec 7169: Secondary ZDDP," 2000, 1 page.  
Kagaya, Mineo, and Sakae Ishikawa. An evaluation and optimization of lubricants for turbocharged gasoline engines. No. 840261. SAE Technical Paper, 1984.  
Ethyl Product Data Sheet "HiTec 611: Overbase Calcium Sulphonate Detergent," 1991, 2 pages.  
The Afton Chemical Grease Portfolio, "Grease," Afton Chemical Corporation, 2016, 12 pages.  
International Search Report and Written Opinion; dated Feb. 9, 2018 for PCT Application No. PCT/US2017/060957.  
Final Office Action; dated Jan. 16, 2018 for U.S. Appl. No. 15/409,513.  
Non-Final Office Action; dated Dec. 6, 2017 for U.S. Appl. No. 15/147,330.  
Office Communication Concerning Third Party Submission; dated Feb. 22, 2018 for U.S. Appl. No. 15/147,404.  
Non-Final Office Action; dated Feb. 23, 2018 for U.S. Appl. No. 15/147,404.  
Takeuchi, K.; Fujimoto, K.; Hirano, S.; Yamashita, M. "Investigation of Engine Oil Effect on Abnormal Combustion in Turbocharged Direct Injection—Spark Ignition Engines," *SAE, Int. J. Fuels Lubr.*, vol. 5, Issue 3, Nov. 2012 , 8 pages.  
Non-Final Office Action; dated May 11, 2016 for U.S. Appl. No. 15/053,617.  
Non-Final Office Action; dated Dec. 20, 2016 for U.S. Appl. No. 15/147,330.  
Non-Final Office Action; dated Dec. 11, 2018 for U.S. Appl. No. 15/409,509.  
Final Office Action; dated Jan. 11, 2019 for U.S. Appl. No. 15/409,513.  
Final Office Action for U.S. Appl. No. 15/409,509; dated May 29, 2019.  
Communication pursuant to Article 94(3) EPC for European Patent Application No. 16741799.7; dated Apr. 29, 2019.  
Invitation to Respond to Written Opinion for Singapore Patent Application No. 11201800281V; dated May 9, 2019.  
Invitation to Respond to Written Opinion for Singapore Patent Application No. 11201800211R; dated May 9, 2019.  
Invitation to Respond to Written Opinion for Singapore Patent Application No. 11201800261P; dated May 9, 2019.  
First Background Requirement Report for Mexican Patent Application No. MX/a/2018/000154; dated Jun. 12, 2019; (Machine Translation).  
Non Final Office Action for U.S. Appl. No. 15/409,503; dated Jan. 8, 2019.  
Final Office Action for U.S. Appl. No. 15/147,375; dated Feb. 21, 2019.  
Non Final Office Action for U.S. Appl. No. 15/409,516; dated Jan. 23, 2019.  
Written Opinion for Singapore Patent Application No. 11201800205T; dated Mar. 12, 2019.  
Written Opinion for Singapore Patent Application No. 11201800279V; dated Mar. 12, 2019.  
Final Office Action for U.S. Appl. No. 15/147,464; dated Apr. 30, 2019.  
Non-Final Office Action for U.S. Appl. No. 16/510,056 dated Oct. 15, 2019; (13 pages).  
Notice of Rejection for Japanese Application No. 2018-501894; dated Oct. 8, 2019 (6 pages).  
Notice of Rejection for Japanese Application No. 2018-543652; dated Oct. 15, 2019 (7 pages).  
Notice of Reasons for Rejection for Japanese Application No. 2017-567100; dated Oct. 8, 2019 (7 pages).  
Notice of Feedback for Korean Application No. 10-2019-7023694; dated Nov. 19, 2019; Machine Translation (21 pages).  
Communication Pursuant to Article 94(3) EPC for corresponding European Application No. 16741797.1; dated Aug. 21, 2019 (3 pages).  
Notice of Grounds for Rejection for corresponding Korean Application No. 10-2018-7003414; dated Sep. 17, 2019 (12 pages).  
Office Action for Canadian application No. 3,050,431; dated Nov. 13, 2019 (4 pages).  
Invitation to Respond to Written Opinion for Singaporean application No. 11201809675U; dated Dec. 26, 2019 (7 pages).  
Invitation to Respond to Written Opinion for Singaporean application No. 11201806979X; dated Dec. 17, 2019 (9 pages).  
Official Action for Russian application No. 2018104014; dated Dec. 23, 2019 (17 pages).  
Official Action for Russian application No. 2018104083; dated Dec. 23, 2019 (13 pages).  
Official Action for Russian application No. 2018104033; dated Dec. 23, 2019 (13 pages).  
Official Action for Russian application No. 2018104035; dated Dec. 25, 2019 (14 pages).  
Official Action for Russian application No. 2018103729; dated Dec. 26, 2019 (14 pages).  
First Office Action for Chinese application No. 201780087217.2; dated Jan. 3, 2020 (11 pages).  
Notice of Rejection for Japanese application No. 2019-538178; dated Jan. 14, 2020 (1 page).  
Notice of Rejection for Japanese application No. 2019-538196; dated Jan. 14, 2020 (2 pages).  
Notice of Rejection for Japanese application No. 2019-538244; dated Jan. 14, 2020 (1 page).  
Notice of Grounds for Rejection for Korean application No. 10-2019-7023837; dated Jan. 21, 2020 (8 pages).  
Notice of Grounds for Rejection for Korean application No. 10-2018-7003363; dated Jan. 21, 2020 (15 pages).  
Notice of Grounds for Rejection for Korean application No. 10-2019-7023661; dated Jan. 21, 2020 (11 pages).  
Written Opinion for Brazilian application No. BR112018000353; dated Feb. 14, 2020 (6 pages).  
Written Opinion for Brazilian application No. BR112018000657; dated Feb. 14, 2020 (6 pages).  
Written Opinion for Brazilian application No. BR112018000615; dated Feb. 14, 2020 (6 pages).  
Written Opinion for Brazilian application No. BR112017028384; dated Feb. 10, 2020 (6 pages).  
Written Opinion for Brazilian application No. BR112018000378; dated Feb. 14, 2020 (6 pages).  
First Office Action for Chinese Application No. 201680039372.2; dated Jun. 12, 2020 (22 pages).  
First Office Action for Chinese Application No. 201680051360.1; dated May 20, 2020 (22 pages).  
First Office Action for Chinese Application No. 201680039322.4; dated May 28, 2020 (15 pages).  
First Office Action for Chinese Application No. 201680039287.6; dated Jun. 10, 2020 (16 pages).  
Examination Report for Indian application No. 201817003275; dated May 12, 2020 (6 pages).  
Examination Report for Indian application No. 201817003462; dated May 15, 2020 (6 pages).  
Examination Report for Indian application No. 201817003464; dated May 15, 2020 (5 pages).

(56)

**References Cited****OTHER PUBLICATIONS**

- Notice of Reasons for Refusal for Japanese application No. 2018-500634; dated Mar. 5, 2020 (15 pages).
- Notification of Reason for Refusal for Korean application No. 10-2018-7003417; dated Feb. 20, 2020 (20 pages).
- Substantive Examination for Mexican application No. MX/a/2018/000153; dated Feb. 5, 2020 (9 pages).
- Written Opinion for Singaporean application No. 11201800205T; dated May 9, 2020 (7 pages).
- First Office Action for Chinese application No. 201780087556.0; dated Mar. 17, 2020 (16 pages).
- Communication pursuant to Article 94(3) EPC for European application No. 17801302.5; dated Jul. 2, 2020 (5 pages).
- Notice of Grounds for Rejection for Korean application No. 10-2019-7023694; dated Mar. 26, 2020 (6 pages).
- Communication pursuant to Article 94(3) EPC for European application No. 17801303.3 dated Jun. 30, 2020 (6 pages).
- First Office Action for Chinese application No. 201780086843.X; dated Feb. 25, 2020 (13 pages).
- Non-Final Office Action for U.S. Appl. No. 16/510,056; dated Apr. 30, 2020 (16 pages).
- Wang Zhi et al., "Research progress of pre-ignition and super-knock in boost gasoline engine", Journal of Automotive Safety and Energy, 6.1 (2015): 17-29 (Machine Translation).
- Invitation to Respond to Written Opinion for corresponding Singaporean application No. 11201809675U; dated May 12, 2021 (6 pages).
- Notification of Reason for Refusal for corresponding Korean application No. 10-2018-7033558; dated May 4, 2021 (21 pages) Machine Translation.
- First Office Action for Chinese application No. 201680051145.1; dated Jul. 29, 2020 (20 pages).
- Second Office Action for Chinese application No. 201680051145.1; dated Apr. 2, 2021 (20 pages).
- Written Opinion for Singaporean application No. 11201806979X; dated Apr. 8, 2021 (6 pages).
- Final Rejection for U.S. Appl. No. 16/510,056; dated Sep. 21, 2020 (12 pages).
- Second office Action for Chinese application No. 201680039287.6; dated Dec. 8, 2020 (16 pages).
- Notice of Rejection for Japanese application No. 2018-500776; dated Aug. 11, 2020 (15 pages).
- Second Office Action for Chinese application No. 201780087556.0; dated Sep. 16, 2020 (6 pages).
- Reason for Refusal for Korean application No. 10-2018-7003366; dated Feb. 24, 2021 (20 pages).
- Second Office Action for Chinese application No. 201680039372.2; dated Mar. 4, 2021 (12 pages).
- Notification of the Decision to Grant for Chinese application No. 201680039287.6; dated Apr. 23, 2021 (9 pages).
- Notice of Rejection for Japanese application No. 2018-500785; dated Aug. 25, 2020 (19 pages).
- Notice of Reasons for Refusal for Japanese application No. 2018-555253; dated Nov. 17, 2020 (9 pages).
- First Office Action for Chinese application No. 201780012112.0; dated Feb. 26, 2021 (22 pages).
- Non-Final Rejection for U.S. Appl. No. 16/510,056; dated Apr. 29, 2021 (16 pages).
- First Office Action for corresponding Chinese application No. 201780026721.1; dated Jun. 3, 2021 (17 pages).
- Communication of Notice of Opposition for European application No. 16741797.1; dated May 31, 2021 (19 pages).

\* cited by examiner

## LUBRICANTS FOR USE IN BOOSTED ENGINES

## TECHNICAL FIELD

The disclosure relates to lubricant compositions having improved resistance to the formation of engine deposits, including turbocharger deposits, when used in a boosted internal combustion engine.

## BACKGROUND

Turbocharged or supercharged engines (i.e. boosted or forced induction internal combustion engines) experience very high operating temperatures. The lubricants used in these engines are exposed to extreme conditions when the engine is stopped, and the lubricant sits in a hot turbocharger as it cools. A lubricant in this environment is prone to the formation of hard deposits in the turbocharger. This phenomenon causes a significant deterioration of turbocharger efficiency which has the potential to cause poor performance and/or severe damage to the engine.

Several published studies have demonstrated that turbocharger use, engine design, engine coatings, piston shape, fuel choice, and/or engine oil additives may contribute to the formation of these deposits in turbocharged engines. Accordingly, there is a need for engine oil additive components and/or combinations that are effective to reduce or prevent the formation of deposits in turbocharged gasoline engines.

Recent specifications such as the 2015 version of the General Motors dexos1® specification, require passage of a Turbocharger Coking Test. One parameter to determine a passing result in the General Motors dexos1® Turbocharger Coking Test is maintaining a percent increase to less than a 13% increase in the Turbo Coolant Outside (TCO) Temperature from the 100 cycle TCO Temperature to the 1800 cycle TCO temperature.

There is a need to improve on a simple pass of the 2015 version of the General Motors dexos1® Turbocharger Coking Test to provide lubricating oil compositions that can score pass ratings of only a 9.0% increase in the Turbo Coolant Outside (TCO) Temperature from the 100 cycle TCO Temperature to the 1800 cycle TCO temperature. “TCO Temperature Increase” as used herein refers to the percent increase in the TCO Temperature from the 100 cycle TCO Temperature to the 1800 cycle TCO temperature as defined by the formula:

$$\frac{(1800 \text{ cycle TCO Temperature} - 100 \text{ cycle TCO temperature})}{100 \text{ cycle TCO Temperature}} \times 100\%$$

## SUMMARY AND TERMS

The present disclosure relates to a lubricating oil composition and method of operating a boosted internal combustion engine. The lubricating oil composition includes greater than 50 wt. % of a base oil of lubricating viscosity, and calcium, nitrogen, molybdenum and boron. The weight ratio of Ca:N (ppm/ppm) in the lubricating oil composition is greater than 1.3 to less than 3.0, the weight ratio of Ca:Mo (ppm/ppm) in the lubricating oil composition is greater than 6.7 to less than 56.3, and the weight ratio of Ca:B (ppm/ppm) in the lubricating oil composition is greater than 5.0 to less than 9.8. The lubricating oil composition does not contain added magnesium from a magnesium-containing detergent. Moreover, the lubricating oil composition is resis-

tant to deposit formation in the boosted internal combustion engine, as shown by its ability to ensure a TCO Temperature Increase of less than 9.0% as measured using the 2015 version of the General Motors dexos1® Turbocharger Coking Test (TC Test).

In another embodiment, the disclosure provides a method for reducing or preventing the formation of deposits in a boosted internal combustion engine. The method includes a step of lubricating a boosted internal combustion engine 10 with a lubricating oil composition comprising greater than 50 wt. % of a base oil of lubricating viscosity, and calcium, nitrogen, molybdenum and boron, and operating the engine lubricated with the lubricating oil composition. The weight ratio of Ca:N (ppm/ppm) in the lubricating oil composition 15 is greater than 1.3 to less than 3.0, the weight ratio of Ca:Mo (ppm/ppm) in the lubricating oil composition is greater than 6.7 to less than 56.3, and the weight ratio of Ca:B (ppm/ ppm) in the lubricating oil composition is greater than 5.0 to less than 9.8. The lubricating oil composition does not 20 contain added magnesium from a magnesium-containing detergent. By lubricating a boosted internal combustion engine with this lubricating oil composition there will be improved resistance to deposit formation in the boosted internal combustion engine, as shown by its ability to ensure 25 a TCO Temperature Increase of less than 9.0% as measured using the 2015 version of the General Motors dexos1® Turbocharger Coking Test.

In any of the foregoing embodiments, the lubricating oil composition may comprise at least one detergent selected 30 from one or more overbased calcium-containing detergents having a total base number (TBN) of greater than 225 mg KOH/g, measured by the method of ASTM D-2896, and optionally one or more low-based/neutral calcium-containing detergents having a TBN of up to 175 mg KOH/g, 35 measured by the method of ASTM D-2896. In some instances, “overbased” may be abbreviated “OB” and in some instances, “low-based/neutral” may be abbreviated “LB/N.”

In each of the foregoing embodiments, the one or more 40 overbased calcium-containing detergents may be selected from an overbased calcium sulfonate detergent, an overbased calcium phenate detergent, an overbased calcium salicylate detergent and mixtures thereof. In each of the 45 embodiments one of the one or more overbased calcium-containing detergents may be an overbased calcium sulfonate detergent.

In each of the foregoing embodiments, the one or more overbased calcium-containing detergents may provide from 50 about 900 to about 3000 ppm by weight calcium to the lubricating oil composition, based on a total weight of the lubricating oil composition. In each of the foregoing 55 embodiments, the one or more overbased calcium-containing detergents may provide from about 1000 to about 2800 ppm by weight calcium to the lubricating oil composition based on a total weight of the lubricating oil composition, or from about 1300 to about 2500 ppm by weight calcium to the lubricating oil composition based on a total weight of the lubricating oil composition.

In each of the foregoing embodiments, the total TBN of 60 the lubricating oil composition may be at least 6.0 mg KOH/g of the lubricating oil composition as measured by the method of ASTM D-2896, or 6.4 to 12.0 mg KOH/g of the lubricating oil composition, or 6.5 to 12.0 mg KOH/g of the lubricating oil composition, as measured by the method 65 of ASTM D-2896.

In each of the foregoing embodiments, the total amount of magnesium in the lubricating oil composition may be less

than 50 ppm, or less than 25 ppm, or no more than 15 ppm, based on a total weight of the lubricating oil composition.

In each of the foregoing embodiments, the lubricating oil composition may comprise a dispersant. In each of the foregoing embodiments, the dispersant may be a boron-containing dispersant. In each of the foregoing embodiments, the boron-containing dispersant may be present in an amount of 1.0-10 wt. %, based on the total weight of the lubricating oil composition. In each of the foregoing embodiments, the boron-containing dispersant may be present in an amount of 1.0-8.5 wt. %, based on the total weight of the lubricating oil composition.

In each of the foregoing embodiments, the one or more borated compound(s) may be included in the lubricating oil composition in an amount sufficient to provide greater than 50 ppm boron to the lubricating oil composition, or greater than 100 ppm boron, or from greater than 50 ppm to 1000 ppm boron, or greater than 100 ppm to 800 ppm boron, or 110 ppm to 600 ppm boron, or 120 ppm to 500 ppm boron to the lubricating oil composition.

In each of the foregoing embodiments, lubricating oil composition may comprise an oil-soluble molybdenum compound. In some embodiments, the oil-soluble molybdenum compound may be present in an amount sufficient to provide about 0.5 ppm to about 2000 ppm of molybdenum to the lubricating oil composition. In some embodiments, the oil-soluble molybdenum compound may be present in an amount sufficient to provide about 5 ppm to about 300 ppm of molybdenum to the lubricating oil composition.

In each of the foregoing embodiments, the lubricating oil composition may have nitrogen present in an amount of about 500 ppm to about 2500 ppm, or in an amount of about 700 ppm to about 2000 ppm, or about 900 ppm to about 1600 ppm based on a total weight of the lubricating oil composition.

In each of the foregoing embodiments, the lubricating oil may further comprise one or more components selected from the group consisting of friction modifiers, antiwear agents, dispersants, antioxidants, and viscosity index improvers.

In each of the foregoing embodiments, the lubricating oil may include greater than 50% base oil, wherein the base oil may be selected from the group consisting of Group II, Group III, Group IV, Group V base oils, and any combination of two or more of the foregoing, and wherein the greater than 50 wt. % of base oil may be other than diluent oils that arise from provision of additive components or viscosity index improvers in the composition. In each of the foregoing embodiments, the lubricating oil composition may comprise greater than 50 wt. % of a Group II base oil, a Group III base oil or a combination thereof, or greater than 70 wt. %, or greater than 75 wt. %, or greater than 80 wt. %, or greater than 85 wt. %, or greater than 90 wt. % of a Group II base oil, a Group III base oil or a combination thereof, or greater than 97 wt. % of a combination of a Group II base oil and a Group III base oil.

In each of the foregoing embodiments, the weight ratio of Ca:N (ppm/ppm) in the lubricating oil composition may be from 1.4 to 2.8 or from 1.5 to 2.3.

In each of the foregoing embodiments, the weight ratio of Ca:Mo (ppm/ppm) in the lubricating oil composition may be from 6.8 to 45 or from greater than 6.8 to 40.

In each of the foregoing embodiments, the weight ratio of Ca:B (ppm/ppm) in the lubricating oil composition may be from greater than 5.1 to 9.7 or from 5.3 to 8.0.

In each of the foregoing embodiments, the lubricating oil composition may be effective to ensure a TCO Temperature

Increase of less than 8.0% as measured using the 2015 version of the General Motors dexos1® Turbocharger Coking Test, or a TCO Temperature Increase of less than 7.0%, or 0.01% to less than 9.0%, or 0.01% to less than 7.0%, or 0.1% to less than 7.0%, or 1.0% to less than 5.0%, as measured using the 2015 version of the General Motors dexos1® Turbocharger Coking Test.

In each of the foregoing embodiments of the method, the lubricating step lubricates a turbocharger or supercharger 10 components combustion chamber or cylinder walls of a spark-ignited direct injection engine or spark-ignited port fuel injected internal combustion engine provided with a turbocharger or a supercharger, including passages, bushings and other components found in a turbocharger or super- 15 charger.

In each of the foregoing embodiments, the overbased calcium-containing detergent may optionally exclude overbased calcium salicylate detergents.

In each of the foregoing embodiments, the lubricating oil 20 composition may optionally exclude any magnesium-containing detergents or the lubricating oil composition may be free of magnesium.

In each of the foregoing embodiments, the lubricating oil composition may not contain any Group IV base oils.

25 In each of the foregoing embodiments, the lubricating oil composition may not contain any Group V base oils.

The following definitions of terms are provided in order to clarify the meanings of certain terms as used herein.

The terms "oil composition," "lubrication composition," 30 "lubricating oil composition," "lubricating oil," "lubricant composition," "lubricating composition," "fully formulated lubricant composition," "lubricant," "crankcase oil," "crankcase lubricant," "engine oil," "engine lubricant," "motor oil," and "motor lubricant" are considered synonymous, fully interchangeable terminology referring to the 35 finished lubrication product comprising greater than 50 wt. % of a base oil plus a minor amount of an additive composition.

As used herein, the terms "additive package," "additive 40 concentrate," "additive composition," "engine oil additive package," "engine oil additive concentrate," "crankcase additive package," "crankcase additive concentrate," "motor oil additive package," "motor oil concentrate," are considered synonymous, fully interchangeable terminology referring to the 45 portion of the lubricating oil composition excluding the greater than 50 wt. % of base oil stock mixture. The additive package may or may not include the viscosity index improver or pour point depressant.

The term "overbased" relates to metal salts, such as metal 50 salts of sulfonates, carboxylates, salicylates, and/or phenates, wherein the amount of metal present exceeds the stoichiometric amount. Such salts may have a conversion level in excess of 100% (i.e., they may comprise more than 55 100% of the theoretical amount of metal needed to convert the acid to its "normal," "neutral" salt). The expression "metal ratio," often abbreviated as MR, is used to designate the ratio of total chemical equivalents of metal in the overbased salt to chemical equivalents of the metal in a neutral salt according to known chemical reactivity and stoichiometry. In a normal or neutral salt, the metal ratio is one and in an overbased salt, MR, is greater than one. They 60 are commonly referred to as overbased, hyperbased, or superbased salts and may be salts of organic sulfur acids, carboxylic acids, salicylates, and/or phenols. In the present disclosure, the lubricating oil composition may contain one or more overbased metal salts. The one or more overbased metal salts can include an overbased detergent having a TBN

of greater than 225 mg KOH/g. The overbased detergent may be a combination of two or more overbased detergents each having a TBN of greater than 225 mg KOH/g. The one or more overbased detergents can include one or more overbased calcium-containing detergents having a TBN of greater than 225 mg KOH/g measured by the method of ASTM D-2896.

As used herein, the term "hydrocarbyl substituent" or "hydrocarbyl group" or "alkyl group" is used in its ordinary sense, which is well-known to those skilled in the art. Specifically, it refers to a group having a carbon atom directly attached to the remainder of the molecule and having predominantly hydrocarbon character. Examples of hydrocarbyl groups include:

- (a) hydrocarbon substituents, that is, aliphatic (e.g., alkyl or alkenyl), alicyclic (e.g., cycloalkyl, cycloalkenyl) substituents, and aromatic-, aliphatic-, and alicyclic-substituted aromatic substituents, as well as cyclic substituents wherein the ring is completed through another portion of the molecule (e.g., two substituents together form an alicyclic moiety);
- (b) substituted hydrocarbon substituents, that is, substituents containing non-hydrocarbon groups which, in the context of this disclosure, do not alter the predominantly hydrocarbon substituent (e.g., halo (especially chloro and fluoro), hydroxy, alkoxy, mercapto, alkyl-mercaptop, nitro, nitroso, amino, alkylamino, and sulfoxo); and
- (c) hetero substituents, that is, substituents which, while having a predominantly hydrocarbon character, in the context of this disclosure, contain other than carbon in a ring or chain otherwise composed of carbon atoms. Heteroatoms may include sulfur, oxygen, and nitrogen, and encompass substituents such as pyridyl, furyl, thienyl, and imidazolyl. In general, no more than two, for example, no more than one, non-hydrocarbon substituent will be present for every ten carbon atoms in the hydrocarbyl group; typically, there will be no non-hydrocarbon substituents in the hydrocarbyl group.

As used herein, the term "percent by weight", unless expressly stated otherwise, means the percentage the recited component represents to the weight of the entire composition. In addition, all values reported herein using "ppm" refer to ppm by weight of the total weight of the lubricating oil composition unless expressly stated otherwise.

The terms "soluble," "oil-soluble," or "dispersible" used herein may, but does not necessarily, indicate that the compounds or additives are soluble, dissolvable, miscible, or capable of being suspended in the oil in all proportions. The foregoing terms do mean, however, that they are, for instance, soluble, suspendable, dissolvable, or stably dispersible in oil to an extent sufficient to exert their intended effect in the environment in which the oil is employed. Moreover, the additional incorporation of other additives may also permit incorporation of higher levels of a particular additive, if desired.

The term "TBN" as employed herein is used to denote the Total Base Number in mg KOH/g composition as measured by the method of ASTM D-2896.

The term "alkyl" as employed herein refers to straight, branched, cyclic, and/or substituted saturated chain moieties of from about 1 to about 100 carbon atoms.

The term "alkenyl" as employed herein refers to straight, branched, cyclic, and/or substituted unsaturated chain moieties of from about 3 to about 10 carbon atoms.

The term "aryl" as employed herein refers to single and multi-ring aromatic compounds that may include alkyl, alkenyl, alkylaryl, amino, hydroxyl, alkoxy, halo substituents, and/or heteroatoms including, but not limited to, nitrogen, oxygen, and sulfur.

Lubricants, combinations of components, or individual components of the present description may be suitable for use in various types of internal combustion engines. Suitable engine types may include, but are not limited to heavy duty 10 diesel, passenger car, light duty diesel, medium speed diesel, marine engines, or motorcycle engines. An internal combustion engine may be a diesel fueled engine, a gasoline fueled engine, a natural gas fueled engine, a bio-fueled engine, a mixed diesel/biofuel fueled engine, a mixed gasoline/biofuel fueled engine, an alcohol fueled engine, a mixed gasoline/alcohol fueled engine, a compressed natural gas (CNG) fueled engine, or mixtures thereof. A diesel engine may be a compression ignited engine. A diesel engine may be a compression ignited engine with a spark-ignition assist. 15 A gasoline engine may be a spark-ignited engine. An internal combustion engine may also be used in combination with an electrical or battery source of power. An engine so configured is commonly known as a hybrid engine. The internal combustion engine may be a 2-stroke, 4-stroke, or rotary engine. Suitable internal combustion engines include marine diesel engines (such as inland marine), aviation piston engines, low-load diesel engines, and motorcycle, automobile, locomotive, and truck engines.

The internal combustion engine may contain components 30 of one or more of an aluminum-alloy, lead, tin, copper, cast iron, magnesium, ceramics, stainless steel, composites, and/or mixtures thereof. The components may be coated, for example, with a diamond-like carbon coating, a lubricated coating, a phosphorus-containing coating, molybdenum-containing coating, a graphite coating, a nano-particle-containing coating, and/or mixtures thereof. The aluminum-alloy may include aluminum silicates, aluminum oxides, or other ceramic materials. In one embodiment the aluminum-alloy is an aluminum-silicate surface. As used herein, the term "aluminum alloy" is intended to be synonymous with "aluminum composite" and to describe a component or surface comprising aluminum and another component intermixed or reacted on a microscopic or nearly microscopic level, regardless of the detailed structure thereof. This would 35 include any conventional alloys with metals other than aluminum as well as composite or alloy-like structures with non-metallic elements or compounds such with ceramic-like materials.

The lubricating oil composition for an internal combustion engine may be suitable for any engine irrespective of the sulfur, phosphorus, or sulfated ash (ASTM D-874) content. The sulfur content of the engine oil lubricant may be about 1 wt. % or less, or about 0.8 wt. % or less, or about 0.5 wt. % or less, or about 0.3 wt. % or less, or about 0.2 wt. % or less. In one embodiment the sulfur content may be in the range of about 0.001 wt. % to about 0.5 wt. %, or about 0.01 wt. % to about 0.3 wt. %. The phosphorus content may be about 0.2 wt. % or less, or about 0.1 wt. % or less, or about 0.085 wt. % or less, or about 0.08 wt. % or less, or even 40 about 0.06 wt. % or less, about 0.055 wt. % or less, or about 0.05 wt. % or less. In one embodiment the phosphorus content may be about 50 ppm to about 1000 ppm, or about 325 ppm to about 850 ppm. The total sulfated ash content may be about 2 wt. % or less, or about 1.5 wt. % or less, or about 45 1.1 wt. % or less, or about 1 wt. % or less, or about 0.8 wt. % or less, or about 0.5 wt. % or less. In one embodiment the sulfated ash content may be about 0.05 wt. % or less.

% to about 0.9 wt. %, or about 0.1 wt. % or about 0.2 wt. % to about 0.45 wt. %. In another embodiment, the sulfur content may be about 0.4 wt. % or less, the phosphorus content may be about 0.08 wt. % or less, and the sulfated ash is about 1 wt. % or less. In yet another embodiment the sulfur content may be about 0.3 wt. % or less, the phosphorus content is about 0.05 wt. % or less, and the sulfated ash may be about 0.8 wt. % or less. ASTM D-4951 is a test method which covers eight elements and can provide elemental composition data. ASTM D-5185 can be used to determine 22 elements in used and unused lubricating oils and base oils, and can provide screening of used oils for indications of wear.

In one embodiment the lubricating oil composition is an engine oil, wherein the lubricating oil composition may have (i) a sulfur content of about 0.5 wt. % or less, (ii) a phosphorus content of about 0.1 wt. % or less, and (iii) a sulfated ash content of about 1.5 wt. % or less.

In some embodiments, the lubricating oil composition is suitable for use with engines powered by low sulfur fuels, such as fuels containing about 1 to about 5% sulfur. Highway vehicle fuels contain about 15 ppm sulfur (or about 0.0015% sulfur). The lubricating oil composition is suitable for use with boosted internal combustion engines including turbocharged or supercharged internal combustion engines.

Further, lubricants of the present description may be suitable to meet one or more industry specification requirements such as ILSAC GF-3, GF-4, GF-5, GF-6, PC-11, CI-4, CJ-4, CK-4, FA-4, ACEA A1/B1, A2/B2, A3/B3, A3/B4, A5/B5, C1, C2, C3, C4, C5, E4/E6/E7/E9, Euro 5/6, Jaso DL-1, Low SAPS, Mid SAPS, or original equipment manufacturer specifications such as dexos1®, dexos2®, MB-Approval 229.51/229.31, 229.71, 229.3/229.5, VW 502.00, 503.00/503.01, 504.00, 505.00, 506.00/506.01, 507.00, 508.00, 509.00, BMW Longlife-04, Porsche C30, Peugeot Citroën Automobiles B71 2290, B71 2296, B71 2297, B71 2300, B71 2302, B71 2312, B71 2007, B71 2008, Ford WSS-M2C153-H, WSS-M2C930-A, WSS-M2C945-A, WSS-M2C913A, WSS-M2C913-B, WSS-M2C913-C, GM 6094-M, Chrysler MS-6395, or any past or future PCMO or HDD specifications not mentioned herein. In some embodiments for passenger car motor oil (PCMO) applications, the amount of phosphorus in the finished fluid is 1000 ppm or less or 900 ppm or less or 800 ppm or less.

Other hardware may not be suitable for use with the disclosed lubricant. A "functional fluid" is a term which encompasses a variety of fluids including but not limited to tractor hydraulic fluids, power transmission fluids including automatic transmission fluids, continuously variable transmission fluids and manual transmission fluids, hydraulic fluids, including tractor hydraulic fluids, some gear oils, power steering fluids, fluids used in wind turbines, compressors, some industrial fluids, and fluids related to power train components. It should be noted that within each of these fluids such as, for example, automatic transmission fluids, there are a variety of different types of fluids due to the various transmissions having different designs which have led to the need for fluids of markedly different functional characteristics. This is contrasted by the term "lubricating fluid" which is not used to generate or transfer power.

With respect to tractor hydraulic fluids, for example, these fluids are all-purpose products used for all lubricant applications in a tractor except for lubricating the engine. These lubricating applications may include lubrication of gearboxes, power take-off and clutch(es), rear axles, reduction gears, wet brakes, and hydraulic accessories.

When a functional fluid is an automatic transmission fluid, the automatic transmission fluids must have enough friction for the clutch plates to transfer power. However, the friction coefficient of fluids has a tendency to decline due to the temperature effects as the fluid heats up during operation. It is important that the tractor hydraulic fluid or automatic transmission fluid maintain its high friction coefficient at elevated temperatures, otherwise brake systems or automatic transmissions may fail. This is not a function of an engine oil.

Tractor fluids, and for example Super Tractor Universal Oils (STUOs) or Universal Tractor Transmission Oils (UTTOs), may combine the performance of engine oils with transmissions, differentials, final-drive planetary gears, wet-brakes, and hydraulic performance. While many of the additives used to formulate a UTTO or a STUO fluid are similar in functionality, they may have deleterious effect if not incorporated properly. For example, some anti-wear and extreme pressure additives used in engine oils can be extremely corrosive to the copper components in hydraulic pumps. Detergents and dispersants used for gasoline or diesel engine performance may be detrimental to wet brake performance. Friction modifiers specific to quiet wet brake noise, may lack the thermal stability required for engine oil performance. Each of these fluids, whether functional, tractor, or lubricating, are designed to meet specific and stringent manufacturer requirements.

The present disclosure provides novel lubricating oil blends formulated for use as automotive crankcase lubricants. Embodiments of the present disclosure may provide lubricating oils suitable for crankcase applications and having improvements in the following characteristics: air entrainment, alcohol fuel compatibility, antioxidant, anti-wear performance, biofuel compatibility, foam reducing properties, friction reduction, fuel economy, pre-ignition prevention, rust inhibition, sludge and/or soot dispersability, piston cleanliness, deposit formation, turbocharger deposit formation and water tolerance.

Engine oils of the present disclosure may be formulated by the addition of one or more additives, as described in detail below, to an appropriate base oil formulation. The additives may be combined with a base oil in the form of an additive package (or concentrate) or, alternatively, may be combined individually with a base oil (or a mixture of both). The fully formulated engine oil may exhibit improved performance properties, based on the additives added and their respective proportions.

Additional details and advantages of the disclosure will be set forth in part in the description which follows, and/or may be learned by practice of the disclosure. The details and advantages of the disclosure may be realized and attained by means of the elements and combinations particularly pointed out in the appended claims. It is to be understood that both the foregoing general description and the following detailed description are exemplary and explanatory only and are not restrictive of the disclosure, as claimed.

## DETAILED DESCRIPTION

Various embodiments of the disclosure provide a lubricating oil composition and methods that may be used for to reduce or prevent the formation of deposits in a boosted internal combustion engine, including in the components of the turbocharger or supercharger. In particular, boosted internal combustion engines of the present disclosure include turbocharged and supercharged internal combustion engines. The boosted internal combustion engines include

spark-ignited, direct injection and/or spark-ignited, port fuel injection engines. The spark-ignited internal combustion engines may be gasoline engines.

The composition of the invention includes a lubricating oil composition containing a base oil of lubricating viscosity and a particular additive composition. The methods of the present disclosure employ the lubricating oil composition containing the additive composition. As described in more detail below the lubricating oil composition may be surprisingly effective for use in reducing or preventing the formation of carbonaceous deposits in a boosted internal combustion engine, including carbonaceous deposits in the components of the turbocharger or supercharger, lubricated with the lubricating oil composition. Since the deposits act as insulators, the amount of deposits can be measured indirectly by measuring the temperature increase in one of the turbocharger coolant passages. The greater the amount of deposits, the greater that the temperature of the turbocharger coolant will increase during engine use. The lubricating oil composition of the present invention is effective to ensure a TCO Temperature Increase of less than 9.0% as measured using the 2015 version of the General Motors dexos1® Turbocharger Coking Test.

In another embodiment, the disclosure provides a method for reducing or preventing the formation of deposits in a boosted internal combustion engine. The method includes a step of lubricating the boosted internal combustion engine with a lubricating oil composition including greater than 50 wt. % of a base oil of lubricating viscosity, and calcium, nitrogen, molybdenum and boron, and operating the engine lubricated with the lubricating oil composition. The weight ratio of Ca:N (ppm/ppm) in the lubricating oil composition is greater than 1.3 to less than 3.0, the weight ratio of Ca:Mo (ppm/ppm) in the lubricating oil composition is greater than 6.7 to less than 56.3, and the weight ratio of Ca:B (ppm/ppm) in the lubricating oil composition is greater than 5.0 to less than 9.8. The lubricating oil composition does not contain added magnesium from a magnesium-containing detergent. By lubricating a boosted internal combustion engine, including the components of the turbocharger or supercharger, with this lubricating oil composition there will be improved resistance to deposit formation in the boosted internal combustion engine, as shown by its ability to ensure a TCO Temperature Increase of less than 9.0% as measured using the 2015 version of the General Motors dexos1® Turbocharger Coking Test. The boosted internal combustion engine is operated and lubricated with the lubricating oil composition whereby the amount of deposits in the engine, including in the components of the turbocharger or supercharger, lubricated with the lubricating oil composition may be reduced or prevented.

In some embodiments of the method, the combustion chamber or cylinder walls of a spark-ignited direct injection engine or spark-ignited port fuel injected internal combustion engine provided with a turbocharger or a supercharger, as well as the passages, bushings and other components of the turbocharger or supercharger are lubricated with the lubricating oil composition and the lubricated spark-ignited direct injection engine is operated whereby the deposits in the engine lubricated with the lubricating oil composition may be reduced or prevented.

In some embodiments of the disclosure, the lubricating oil composition has improved resistance to deposit formation in the boosted internal combustion engine, as shown by its ability to ensure a TCO Temperature Increase of less than 9.0% as measured using the 2015 version of the General Motors dexos1® Turbocharger Coking Test. In some

embodiments, the lubricating oil composition may be effective to ensure a TCO Temperature Increase of less than 8.0% as measured using the 2015 version of the General Motors dexos1® Turbocharger Coking Test, or a TCO Temperature Increase of less than 5.0% as measured using the 2015 version of the General Motors dexos1® Turbocharger Coking Test.

The calcium in the lubricating oil composition may be provided by various sources including detergents. In some embodiments, the lubricating oil composition may comprise at least one detergent selected from one or more overbased calcium-containing detergents having a TBN of greater than 225 mg KOH/g, measured by the method of ASTM D-2896, and optionally one or more low-based/neutral calcium-containing detergents having a TBN of up to 175 mg KOH/g, measured by the method of ASTM D-2896.

In some embodiments, the one or more overbased calcium-containing detergents may provide from about 900 to about 3000 ppm by weight calcium to the lubricating oil composition, based on a total weight of the lubricating oil composition, or from about 1000 to about 2800 ppm by weight calcium to the lubricating oil composition based on a total weight of the lubricating oil composition, or from about 1300 to about 2500 ppm by weight calcium to the lubricating oil composition based on a total weight of the lubricating oil composition.

In some embodiments, the weight ratio of Ca:B in the lubricating oil composition may be greater than 5.0 to less than 9.8, or the weight ratio of Ca:B in the lubricating oil composition is greater than 5.1 to 9.7, or the weight ratio of Ca:B in the lubricating oil composition is 5.3 to 8.0.

The lubricating oil composition contains both boron and nitrogen. One source for providing boron and/or nitrogen to the lubricating oil composition is boron-containing dispersants. In some embodiments, the lubricating oil composition may comprise a dispersant which can be a boron-containing dispersant. In some embodiments, the boron-containing dispersant may be present in an amount of 1.0-10 wt. %, based on the total weight of the lubricating oil composition, and even more preferably the boron-containing dispersant may be in an amount of 1.0-8.5 wt. %, based on the total weight of the lubricating oil composition.

The lubricating oil composition of the present invention may have a weight ratio of Ca:N (ppm/ppm) in the lubricating oil composition that is greater than 1.3 to less than 3.0. In some embodiments, the weight ratio of Ca:N (ppm/ppm) in the lubricating oil composition may be from 1.4 to 2.8, or the weight ratio of Ca:N (ppm/ppm) in the lubricating oil composition may be from 1.5 to 2.3.

In some embodiments, the nitrogen may be present in the lubricating oil composition in an amount of about 500 ppm to about 2500 ppm, or about 700 ppm to about 2000 ppm, or about 900 ppm to about 1600 ppm. In some embodiments, the nitrogen present in the lubricant composition can be added as part of one or more of the dispersants, antioxidants and friction modifiers.

The lubricating oil composition of the present invention may have a Ca:Mo weight ratio of from greater than 6.7 to 56.3 or from 6.8 to 45 or from greater than 6.8 to 40.

The lubricating oil compositions of the present invention may have a total TBN of at least 6.0 mg KOH/g of the lubricating oil composition, or 6.4 to 12.0 mg KOH/g of the lubricating oil composition, or 6.5 to 12.0 mg KOH/g of the lubricating oil composition, all as measured by the method of ASTM D-2896.

## Base Oil

The base oil used in the lubricating oil compositions herein may be selected from any of the base oils in Groups I-V as specified in the American Petroleum Institute (API) Base Oil Interchangeability Guidelines. The five base oil groups are as follows:

TABLE 1

| Base oil Category | Sulfur (%)                                          |        | Saturates (%) | Viscosity Index |
|-------------------|-----------------------------------------------------|--------|---------------|-----------------|
| Group I           | >0.03                                               | and/or | <90           | 80 to 120       |
| Group II          | ≤0.03                                               | and    | ≥90           | 80 to 120       |
| Group III         | ≤0.03                                               | and    | ≥90           | ≥120            |
| Group IV          | All polyalpha-olefins (PAOs)                        |        |               |                 |
| Group V           | All others not included in Groups I, II, III, or IV |        |               |                 |

Groups I, II, and III are mineral oil process stocks. Group IV base oils contain true synthetic molecular species, which are produced by polymerization of olefinically unsaturated hydrocarbons. Many Group V base oils are also true synthetic products and may include diesters, polyol esters, polyalkylene glycols, alkylated aromatics, polyphosphate esters, polyvinyl ethers, and/or polyphenyl ethers, and the like, but may also be naturally occurring oils, such as vegetable oils. It should be noted that although Group III base oils are derived from mineral oil, the rigorous processing that these fluids undergo causes their physical properties to be very similar to some true synthetics, such as PAOs. Therefore, oils derived from Group III base oils may be referred to as synthetic fluids in the industry.

The base oil used in the disclosed lubricating oil composition may be a mineral oil, animal oil, vegetable oil, synthetic oil, or mixtures thereof. Suitable oils may be derived from hydrocracking, hydrogenation, hydrofinishing, unrefined, refined, and re-refined oils, and mixtures thereof.

Unrefined oils are those derived from a natural, mineral, or synthetic source without or with little further purification treatment. Refined oils are similar to the unrefined oils except that they have been treated in one or more purification steps, which may result in the improvement of one or more properties. Examples of suitable purification techniques are solvent extraction, secondary distillation, acid or base extraction, filtration, percolation, and the like. Oils refined to the quality of an edible may or may not be useful. Edible oils may also be called white oils. In some embodiments, lubricating oil compositions are free of edible or white oils.

Re-refined oils are also known as reclaimed or reprocessed oils. These oils are obtained similarly to refined oils using the same or similar processes. Often these oils are additionally processed by techniques directed to removal of spent additives and oil breakdown products.

Mineral oils may include oils obtained by drilling or from plants and animals or any mixtures thereof. For example such oils may include, but are not limited to, castor oil, lard oil, olive oil, peanut oil, corn oil, soybean oil, and linseed oil, as well as mineral lubricating oils, such as liquid petroleum oils and solvent-treated or acid-treated mineral lubricating oils of the paraffinic, naphthenic or mixed paraffinic-naphthenic types. Such oils may be partially or fully hydrogenated, if desired. Oils derived from coal or shale may also be useful.

Useful synthetic lubricating oils may include hydrocarbon oils such as polymerized, oligomerized, or interpolymerized olefins (e.g., polybutylenes, polypropylenes, propylene/isobutylene copolymers); poly(1-hexenes), poly(1-octenes), 5 trimers or oligomers of 1-decene, e.g., poly(1-decenes), such materials being often referred to as  $\alpha$ -olefins, and mixtures thereof; alkyl-benzenes (e.g. dodecylbenzenes, tetradecylbenzenes, dinonylbenzenes, di-(2-ethylhexyl)-benzenes); polyphenyls (e.g., biphenyls, terphenyls, alkylated polyphenyls); diphenyl alkanes, alkylated diphenyl alkanes, alkylated diphenyl ethers and alkylated diphenyl sulfides and the derivatives, analogs and homologs thereof or mixtures thereof. Polyalphaolefins are typically hydrogenated materials.

10 Other synthetic lubricating oils include polyol esters, diesters, liquid esters of phosphorus-containing acids (e.g., tricresyl phosphate, trioctyl phosphate, and the diethyl ester of decane phosphonic acid), or polymeric tetrahydrofurans. Synthetic oils may be produced by Fischer-Tropsch reactions and typically may be hydroisomerized Fischer-Tropsch hydrocarbons or waxes. In one embodiment oils may be prepared by a Fischer-Tropsch gas-to-liquid synthetic procedure as well as other gas-to-liquid oils.

15 The greater than 50 wt. % of base oil included in a lubricating composition may be selected from the group consisting of Group I, Group II, a Group III, a Group IV, a Group V, and a combination of two or more of the foregoing, and wherein the greater than 50 wt. % of base oil is other than base oils that arise from provision of additive components or viscosity index improvers in the composition. In another embodiment, the greater than 50 wt. % of base oil included in a lubricating composition may be selected from the group consisting of Group II, a Group III, a Group IV, a Group V, and a combination of two or more of the foregoing, 20 and wherein the greater than 50 wt. % of base oil is other than diluent oils that arise from provision of additive components or viscosity index improvers in the composition.

25 The amount of the oil of lubricating viscosity present may be the balance remaining after subtracting from 100 wt. % the sum of the amount of the performance additives inclusive of viscosity index improver(s) and/or pour point depressant(s) and/or other top treat additives. For example, the oil of lubricating viscosity that may be present in a finished fluid may be a major amount, such as greater than about 50 wt. %, greater than about 60 wt. %, greater than about 70 wt. %, greater than about 80 wt. %, greater than about 85 wt. %, or greater than about 90 wt. %, all based on the total weight of the lubricating oil composition.

30 The lubricating oil composition may comprise not more than 10 wt. % of a Group IV base oil, a Group V base oil, or a combination thereof. In each of the foregoing embodiments, the lubricating oil compositions may comprise less than 5 wt. % of a Group V base oil. In some embodiments, the lubricating oil composition does not contain any Group IV base oils and/or the lubricating oil composition does not contain any Group V base oils.

## Detergents

35 The lubricating oil composition may comprise one or more detergents, subject to the constraint that no magnesium may be added to the lubricating oil compositions by a magnesium-containing detergent. In some embodiments, the lubricating oil composition may comprise one or more overbased calcium-containing detergents and optionally other detergents. Suitable detergent substrates include phenates, sulfur containing phenates, sulfonates, calixarates, salixarates, salicylates, carboxylic acids, phosphorus acids, mono- and/or di-thiophosphoric acids, alkyl phenols, sulfur

coupled alkyl phenol compounds, or methylene bridged phenols. Suitable detergents and their methods of preparation are described in greater detail in numerous patent publications, including U.S. Pat. No. 7,732,390 and references cited therein. The detergent substrate may be salted with an alkali or alkaline earth metal such as, but not limited to, calcium, potassium, sodium, lithium, barium, or mixtures thereof. In some embodiments, the detergent is free of barium.

A suitable detergent may include alkali or alkaline earth metal salts of petroleum sulfonic acids and long chain mono- or di-alkylarylsulfonic acids with the aryl group being benzyl, tolyl, and xylyl. Examples of suitable additional detergents include, but are not limited to, calcium phenates, calcium sulfur containing phenates, calcium sulfonates, calcium calixarates, calcium salixarates, calcium salicylates, calcium carboxylic acids, calcium phosphorus acids, calcium mono- and/or di-thiophosphoric acids, calcium alkyl phenols, calcium sulfur coupled alkyl phenol compounds, calcium methylene bridged phenols sodium phenates, sodium sulfur containing phenates, sodium sulfonates, sodium calixarates, sodium salixarates, sodium salicylates, sodium carboxylic acids, sodium phosphorus acids, sodium mono- and/or di-thiophosphoric acids, sodium alkyl phenols, sodium sulfur coupled alkyl phenol compounds, or sodium methylene bridged phenols.

Overbased detergents are well known in the art and may be alkali or alkaline earth metal overbased detergents. Such detergents may be prepared by reacting a metal oxide or metal hydroxide with a substrate and carbon dioxide gas. The substrate is typically an acid, for example, an acid such as an aliphatic substituted sulfonic acid, an aliphatic substituted carboxylic acid, or an aliphatic substituted phenol.

The terminology "overbased" relates to metal salts, such as metal salts of sulfonates, carboxylates, and phenates, wherein the amount of metal present exceeds the stoichiometric amount. Such salts may have a conversion level in excess of 100% (i.e., they may comprise more than 100% of the theoretical amount of metal needed to convert the acid to its "normal," "neutral" salt). The expression "metal ratio," often abbreviated as MR, is used to designate the ratio of total chemical equivalents of metal in the overbased salt to chemical equivalents of the metal in a neutral salt according to known chemical reactivity and stoichiometry. In a normal or neutral salt, the metal ratio is 1 and in an overbased salt, MR, is greater than 1. They are commonly referred to as overbased, hyperbased, or superbased salts and may be salts of organic sulfur acids, carboxylic acids, or phenols.

An overbased detergent may have a TBN of greater 225 mg KOH/gram, or as further examples, an overbased detergent may have a TBN of about 250 mg KOH/gram or greater, or a TBN of about 300 mg KOH/gram or greater, or a TBN of about 350 mg KOH/gram or greater, or a TBN of about 375 mg KOH/gram or greater, or a TBN of about 400 mg KOH/gram or greater, as measured by the method of ASTM D-2896.

Examples of suitable overbased detergents include, but are not limited to, overbased calcium phenates, overbased calcium sulfur containing phenates, overbased calcium sulfonates, overbased calcium calixarates, overbased calcium salixarates, overbased calcium salicylates, overbased calcium carboxylic acids, overbased calcium phosphorus acids, overbased calcium mono- and/or di-thiophosphoric acids, overbased calcium alkyl phenols, overbased calcium sulfur coupled alkyl phenol compounds, and overbased calcium methylene bridged phenols.

The overbased detergent may have a metal to substrate ratio of from 1.1:1, or from 2:1, or from 4:1, or from 5:1, or from 7:1, or from 10:1.

In some embodiments, a detergent is effective at reducing or preventing rust in an engine.

The total detergent may be present at up to 10 wt. %, or about up to 8 wt. %, or up to about 4 wt. %, or greater than about 1 wt. % to about 8 wt. %, or greater than about 1 wt. % to about 4 wt. %, based on a total weight of the lubricating oil composition.

The total detergent may be present in an amount to provide from about 950 to about 3500 ppm metal to the finished fluid. In other embodiments, the detergent may provide from about 1100 to about 3000 ppm of metal, or about 1150 to about 2500 ppm of metal, or about 1200 to about 2400 ppm of metal to the finished fluid.

In some embodiments, the lubricating oil compositions of the present disclosure comprise at least one detergent selected from one or more overbased calcium-containing detergents having a TBN of greater than 225 mg KOH/g, measured by the method of ASTM D-2896, and optionally one or more low-based/neutral calcium-containing detergents having a TBN of up to 175 mg KOH/g, measured by the method of ASTM D-2896. The present disclosure also includes methods of using such lubricating oil compositions in a method or lubricating an engine by lubricating the engine with the lubricating oil composition and operating the engine.

The lubricating oil composition of the disclosure may have a total amount of calcium from the overbased calcium-containing detergent that ranges from 900 ppm by weight to about 3000 ppm by weight based on a total weight of the lubricating oil composition. The overbased calcium-containing detergent may be selected from an overbased calcium sulfonate detergent, an overbased calcium phenate detergent, and an overbased calcium salicylate detergent. In certain embodiments, the overbased calcium-containing detergent comprises an overbased calcium sulfonate detergent. In certain embodiments, the overbased detergent is one or more calcium-containing detergents. Preferably the overbased detergent is a calcium sulfonate detergent.

In certain embodiments, the one or more overbased calcium-containing detergents provide from about 900 to about 2800 ppm calcium to the finished fluid. As a further example, the one or more overbased calcium-containing detergents may be present in an amount to provide from about 1300 to about 2500 ppm calcium.

In the present invention, the lubricating oil composition does not contain added magnesium from a magnesium-containing detergent, i.e., a detergent having a metal that is primarily (greater than 95 mole %) magnesium. The total amount of magnesium in the lubricating oil composition may be less than 50 ppm, or less than 25 ppm, or no more than 15 ppm.

The lubricating oil compositions of the present invention may optionally also contain one or more low-based/neutral detergents. The low-based/neutral detergent has a TBN of up to 175 mg KOH/g, or up to 150 mg KOH/g. The low-based/neutral detergent may include a calcium-containing detergent. The low-based/neutral calcium-containing detergent may be selected from a calcium sulfonate detergent, a calcium phenate detergent and a calcium salicylate detergent. In some embodiments, the low-based/neutral detergent may be a calcium-containing detergent or a mixture of calcium-containing detergents. In some embodiments, the low-based/neutral detergent may be a calcium sulfonate

## 15

detergent or a calcium phenate detergent. In some embodiments, the lubricating oil composition does not contain a low-based/neutral detergent.

The low-based/neutral detergent, when present, may comprise at least 0.2 wt. % of the lubricating oil composition. In some embodiments, the low-based/neutral detergent may comprise at least 0.25 wt. %, or at least 0.5 wt. %, or at least 0.7 wt. %, or at least 1.0 wt. % or at least 1.2 wt. % or at least 2.0 wt. % of the lubricating oil composition. The low-based/neutral detergent may optionally include one or more low-based/neutral calcium-containing detergents.

In certain embodiments, the one or more low-based/neutral calcium-containing detergents may provide from about 50 to about 1000 ppm calcium by weight to the lubricating oil composition based on a total weight of the lubricating oil composition. In some embodiments, the one or more low-based/neutral calcium-containing detergents may provide from 75 to less than 800 ppm, or from 100 to 600 ppm, or from 125 to 500 ppm by weight calcium to the lubricating oil composition based on a total weight of the lubricating oil composition.

In some embodiments the ratio of the ppm of calcium, by weight, provided to the lubricating oil composition by the low-based/neutral detergent to the ppm of calcium, by weight, provided to the lubricating oil composition by the overbased calcium detergent, may be from 0 to about 1, or from about 0.03 to about 0.7, or from about 0.05 to about 0.5, or from about 0.08 to about 0.4.

The overbased calcium-containing detergent may be an overbased calcium sulfonate detergent. The overbased calcium-containing detergent may optionally exclude overbased calcium salicylate detergents. The lubricating oil excludes any magnesium-containing detergents or is free of magnesium. In any of the embodiments of the disclosure, the amount of sodium in the lubricating composition may be limited to not more than 150 ppm of sodium, or 100 ppm of sodium, or 50 ppm of sodium, based on a total weight of the lubricating oil composition.

## Molybdenum-Containing Component

The lubricating oil compositions herein contain molybdenum and this molybdenum may be provided to the lubricating oil composition in the form of one or more molybdenum-containing compounds. An oil-soluble molybdenum compound may have the functional performance of an antiwear agent, an antioxidant, a friction modifier, or mixtures thereof. An oil-soluble molybdenum compound may include molybdenum dithiocarbamates, molybdenum dialkyldithiophosphates, molybdenum dithiophosphinates, amine salts of molybdenum compounds, molybdenum xanthates, molybdenum thioxanthates, molybdenum sulfides, molybdenum carboxylates, molybdenum alkoxides, a tri-nuclear organo-molybdenum compound, and/or mixtures thereof. The molybdenum sulfides include molybdenum disulfide. The molybdenum disulfide may be in the form of a stable dispersion. In one embodiment the oil-soluble molybdenum compound may be selected from the group consisting of molybdenum dithiocarbamates, molybdenum dialkyldithiophosphates, amine salts of molybdenum compounds, and mixtures thereof. In one embodiment the oil-soluble molybdenum compound may be a molybdenum dithiocarbamate.

Suitable examples of molybdenum compounds which may be used include commercial materials sold under the trade names such as Molyvan 822<sup>TM</sup>, Molyvan<sup>TM</sup> A, Molyvan 2000<sup>TM</sup> and Molyvan 855<sup>TM</sup> from R. T. Vanderbilt Co., Ltd., and Sakura-Lube<sup>TM</sup> S-165, S-200, S-300, S-310G, S-525, S-600, S-700, and S-710 available from Adeka

## 16

Corporation, and mixtures thereof. Suitable molybdenum components are described in U.S. Pat. No. 5,650,381; U.S. RE 37,363 E1; U.S. RE 38,929 E1; and U.S. RE 40,595 E1.

Additionally, the molybdenum compound may be an acidic molybdenum compound. Included are molybdic acid, ammonium molybdate, sodium molybdate, potassium molybdate, and other alkaline metal molybdates and other molybdenum salts, e.g., hydrogen sodium molybdate,  $\text{MoOCl}_4$ ,  $\text{MoO}_2\text{Br}_2$ ,  $\text{Mo}_2\text{O}_3\text{Cl}_6$ , molybdenum trioxide or similar acidic molybdenum compounds. Alternatively, the compositions can be provided with molybdenum by molybdenum/sulfur complexes of basic nitrogen compounds as described, for example, in U.S. Pat. Nos. 4,263,152; 4,285,822; 4,283,295; 4,272,387; 4,265,773; 4,261,843; 4,259,195 and 4,259,194; and U.S. Patent Publication No. 2002/0038525.

Another class of suitable organo-molybdenum compounds are trinuclear molybdenum compounds, such as those of the formula  $\text{Mo}_3\text{S}_k\text{L}_n\text{Q}_z$  and mixtures thereof, wherein S represents sulfur, L represents independently selected ligands having organo groups with a sufficient number of carbon atoms to render the compound soluble or dispersible in the oil, n is from 1 to 4, k varies from 4 through 7, Q is selected from the group of neutral electron donating compounds such as water, amines, alcohols, phosphines, and ethers, and z ranges from 0 to 5 and includes non-stoichiometric values. At least 21 total carbon atoms may be present among all the ligands' organo groups, such as at least 25, at least 30, or at least 35 carbon atoms. Additional suitable molybdenum compounds are described in U.S. Pat. No. 6,723,685.

The oil-soluble molybdenum compound may be present in an amount sufficient to provide about 0.5 ppm to about 2000 ppm, about 1 ppm to about 700 ppm, about 1 ppm to about 550 ppm, about 5 ppm to about 300 ppm, or about 20 ppm to about 250 ppm of molybdenum to the lubricating oil composition based on the total weight of the lubricating composition.

## Boron-Containing Compounds

The lubricating oil compositions herein contain boron which may be provided to the lubricating oil composition in the form of one or more boron-containing compounds such as boron-containing dispersants as discussed above.

Examples of boron-containing compounds include borate esters, borated fatty amines, borated epoxides, borated detergents, and borated dispersants, such as borated succinimide dispersants, as disclosed in U.S. Pat. No. 5,883,057.

The one or more boron-containing compounds can be used in an amount sufficient to provide about 0.01 wt. % to about 10 wt. %, about 0.05 wt. % to about 8.5 wt. %, or about 0.1 wt. % to about 3 wt. % of the lubricating oil composition, based on the total weight of the lubricating composition. The one or more boron-containing compounds may be included in the lubricating oil composition in an amount sufficient to provide greater than 50 ppm boron to the lubricating oil composition, or greater than 100 ppm boron, or from greater than 50 ppm to 1000 ppm boron, or greater than 100 ppm to 800 ppm boron, or 110 ppm to 600 ppm boron, or 120 ppm to 500 ppm boron to the lubricating oil composition, based on the total weight of the lubricating composition.

The lubricating oil composition may also include one or more optional components selected from the various additives set forth below.

## Antioxidants

The lubricating oil compositions herein also may optionally contain one or more antioxidants. Antioxidant com-

pounds are known and include for example, phenates, phenate sulfides, sulfurized olefins, phosphosulfurized terpenes, sulfurized esters, aromatic amines, alkylated diphenylamines (e.g., nonyl diphenylamine, di-nonyl diphenylamine, octyl diphenylamine, di-octyl diphenylamine), phenyl-alpha-naphthylamines, alkylated phenyl-alpha-naphthylamines, hindered non-aromatic amines, phenols, hindered phenols, oil-soluble molybdenum compounds, macromolecular antioxidants, or mixtures thereof. Antioxidant compounds may be used alone or in combination.

The hindered phenol antioxidant may contain a secondary butyl and/or a tertiary butyl group as a sterically hindering group. The phenol group may be further substituted with a hydrocarbyl group and/or a bridging group linking to a second aromatic group. Examples of suitable hindered phenol antioxidants include 2,6-di-tert-butylphenol, 4-methyl-2,6-di-tert-butylphenol, 4-ethyl-2,6-di-tert-butylphenol, 4-propyl-2,6-di-tert-butylphenol or 4-butyl-2,6-di-tert-butylphenol, or 4-dodecyl-2,6-di-tert-butylphenol. In one embodiment the hindered phenol antioxidant may be an ester and may include, e.g., IRGANOX<sup>TM</sup> L-135 available from BASF or an addition product derived from 2,6-di-tert-butylphenol and an alkyl acrylate, wherein the alkyl group may contain about 1 to about 18, or about 2 to about 12, or about 2 to about 8, or about 2 to about 6, or about 4 carbon atoms. Another commercially available hindered phenol antioxidant may be an ester and may include ETHANOX<sup>TM</sup> 4716 available from Albemarle Corporation.

Useful antioxidants may include diarylamines and high molecular weight phenols. In an embodiment, the lubricating oil composition may contain a mixture of a diarylamine and a high molecular weight phenol, such that each antioxidant may be present in an amount sufficient to provide up to about 5%, by weight, based upon the total weight of the lubricating oil composition. In an embodiment, the antioxidant may be a mixture of about 0.3 to about 1.5% diarylamine and about 0.4 to about 2.5% high molecular weight phenol, by weight, based upon the total weight of the lubricating oil composition.

Examples of suitable olefins that may be sulfurized to form a sulfurized olefin include propylene, butylene, isobutylene, polyisobutylene, pentene, hexene, heptene, octene, nonene, decene, undecene, dodecene, tridecene, tetradecene, pentadecene, hexadecene, heptadecene, octadecene, nonadecene, eicosene or mixtures thereof. In one embodiment, hexadecene, heptadecene, octadecene, nonadecene, eicosene or mixtures thereof and their dimers, trimers and tetramers are especially useful olefins. Alternatively, the olefin may be a Diels-Alder adduct of a diene such as 1,3-butadiene and an unsaturated ester, such as, butylacrylate.

Another class of sulfurized olefin includes sulfurized fatty acids and their esters. The fatty acids are often obtained from vegetable oil or animal oil and typically contain about 4 to about 22 carbon atoms. Examples of suitable fatty acids and their esters include triglycerides, oleic acid, linoleic acid, palmitoleic acid or mixtures thereof. Often, the fatty acids are obtained from lard oil, tall oil, peanut oil, soybean oil, cottonseed oil, sunflower seed oil or mixtures thereof. Fatty acids and/or ester may be mixed with olefins, such as  $\alpha$ -olefins.

The one or more antioxidant(s) may be present in ranges about 0 wt. % to about 5.0 wt. %, or about 0.1 wt. % to about 4.0 wt. %, or about 0.5 wt. % to about 3 wt. %, of the lubricating oil composition, based on the total weight of the lubricating composition.

#### Antiwear Agents

The lubricating oil compositions herein also may optionally contain one or more antiwear agents. Examples of suitable antiwear agents include, but are not limited to, a metal thiophosphate; a metal dialkyldithiophosphate; a phosphoric acid ester or salt thereof a phosphate ester(s); a phosphite; a phosphorus-containing carboxylic ester, ether, or amide; a sulfurized olefin; thiocarbamate-containing compounds including, thiocarbamate esters, alkylene-coupled thiocarbamates, and bis(S-alkyldithiocarbamyl)disulfides; and mixtures thereof. A suitable antiwear agent may be a molybdenum dithiocarbamate. The phosphorus containing antiwear agents are more fully described in European Patent 612 839. The metal in the dialkyl dithiophosphate salts may be an alkali metal, alkaline earth metal, aluminum, lead, tin, molybdenum, manganese, nickel, copper, titanium, or zinc. A useful antiwear agent may be zinc dialkyldithiophosphate.

Further examples of suitable antiwear agents include 20 titanium compounds, tartrates, tartrimides, oil soluble amine salts of phosphorus compounds, sulfurized olefins, phosphites (such as dibutyl phosphite), phosphonates, thiocarbamate-containing compounds, such as thiocarbamate esters, thiocarbamate amides, thiocarbamic ethers, alkylene-coupled thiocarbamates, and bis(S-alkyldithiocarbamyl)disulfides. The tartrate or tartrimide may contain alkyl-ester groups, where the sum of carbon atoms on the alkyl groups may be at least 8. The antiwear agent may in one embodiment include a citrate.

30 The antiwear agent may be present in ranges including about 0 wt. % to about 10 wt. %, or about 0.01 wt. % to about 8 wt. %, or about 0.05 wt. % to about 5 wt. %, or about 0.1 wt. % to about 3 wt. % of the lubricating oil composition, based on the total weight of the lubricating composition.

35 An antiwear compound may be a zinc dihydrocarbyl dithiophosphate (ZDDP) having a P:Zn ratio of from about 1:0.8 to about 1:1.7.

#### Dispersants

The lubricating oil composition may optionally further 40 comprise one or more dispersants or mixtures thereof. Dispersants are often known as ashless-type dispersants because, prior to mixing in a lubricating oil composition, they do not contain ash-forming metals and they do not normally contribute any ash when added to a lubricant. 45 Ashless type dispersants are characterized by a polar group attached to a relatively high molecular weight hydrocarbon chain. Typical ashless dispersants include N-substituted long chain alkenyl succinimides. Examples of N-substituted long chain alkenyl succinimides include polyisobutylene succinimide with number average molecular weight of the polyisobutylene substituent in the range about 350 to about 50,000, or to about 5,000, or to about 3,000. Succinimide dispersants and their preparation are disclosed, for instance in U.S. Pat. Nos. 7,897,696 or 4,234,435. The polyolefin 50 may be prepared from polymerizable monomers containing about 2 to about 16, or about 2 to about 8, or about 2 to about 6 carbon atoms. Succinimide dispersants are typically the imide formed from a polyamine, typically a poly(ethyleneamine).

60 In an embodiment the present disclosure further comprises at least one polyisobutylene succinimide dispersant derived from polyisobutylene with number average molecular weight in the range about 350 to about 50,000, or to about 5000, or to about 3000. The polyisobutylene succinimide may be used alone or in combination with other dispersants.

65 In some embodiments, polyisobutylene, when included, may have greater than 50 mol %, greater than 60 mol %,

greater than 70 mol %, greater than 80 mol %, or greater than 90 mol % content of terminal double bonds. Such PIB is also referred to as highly reactive PIB ("HR-PIB"). HR-PIB having a number average molecular weight ranging from about 800 to about 5000 is suitable for use in embodiments of the present disclosure. Conventional PIB typically has less than 50 mol %, less than 40 mol %, less than 30 mol %, less than 20 mol %, or less than 10 mol % content of terminal double bonds.

An HR-PIB having a number average molecular weight ranging from about 900 to about 3000 may be suitable. Such HR-PIB is commercially available, or can be synthesized by the polymerization of isobutene in the presence of a non-chlorinated catalyst such as boron trifluoride, as described in U.S. Pat. No. 4,152,499 to Boerzel, et al. and U.S. Pat. No. 5,739,355 to Gateau, et al. When used in the aforementioned thermal ene reaction, HR-PIB may lead to higher conversion rates in the reaction, as well as lower amounts of sediment formation, due to increased reactivity. A suitable method is described in U.S. Pat. No. 7,897,696.

In one embodiment the present disclosure further comprises at least one dispersant derived from polyisobutylene succinic anhydride ("PIBSA"). The PIBSA may have an average of between about 1.0 and about 2.0 succinic acid moieties per polymer.

The % actives of the alkenyl or alkyl succinic anhydride can be determined using a chromatographic technique. This method is described in column 5 and 6 in U.S. Pat. No. 5,334,321.

The percent conversion of the polyolefin is calculated from the % actives using the equation in column 5 and 6 in U.S. Pat. No. 5,334,321.

Unless stated otherwise, all percentages are in weight percent and all molecular weights are number average molecular weights.

In one embodiment, the dispersant may be derived from a polyalphaolefin (PAO) succinic anhydride.

In one embodiment, the dispersant may be derived from olefin maleic anhydride copolymer. As an example, the dispersant may be described as a poly-PIBSA.

In an embodiment, the dispersant may be derived from an anhydride which is grafted to an ethylene-propylene copolymer.

One class of suitable dispersants may be Mannich bases. Mannich bases are materials that are formed by the condensation of a higher molecular weight, alkyl substituted phenol, a polyalkylene polyamine, and an aldehyde such as formaldehyde. Mannich bases are described in more detail in U.S. Pat. No. 3,634,515.

A suitable class of dispersants may be high molecular weight esters or half ester amides.

A suitable dispersant may also be post-treated by conventional methods by a reaction with any of a variety of agents. Among these are boron, urea, thiourea, dimercaptothiadiazoles, carbon disulfide, aldehydes, ketones, carboxylic acids, hydrocarbon-substituted succinic anhydrides, maleic anhydride, nitriles, epoxides, carbonates, cyclic carbonates, hindered phenolic esters, and phosphorus compounds. U.S. Pat. Nos. 7,645,726; 7,214,649; and 8,048,831 disclose suitable dispersants and posttreatments.

In addition to the carbonate and boric acids post-treatments both the compounds may be post-treated, or further post-treatment, with a variety of post-treatments designed to improve or impart different properties. Such post-treatments include those summarized in columns 27-29 of U.S. Pat. No. 5,241,003. Such treatments include, treatment with:

Inorganic phosphorus acids or anhydrides (e.g., U.S. Pat. Nos. 3,403,102 and 4,648,980);

Organic phosphorus compounds (e.g., U.S. Pat. No. 3,502,677);

Phosphorus pentasulfides;

Boron compounds as already noted above (e.g., U.S. Pat. Nos. 3,178,663 and 4,652,387);

Carboxylic acid, polycarboxylic acids, anhydrides and/or acid halides (e.g., U.S. Pat. Nos. 3,708,522 and 4,948,386);

Epoxides, polyepoxides or thioepoxides (e.g., U.S. Pat. Nos. 3,859,318 and 5,026,495);

Aldehyde or ketone (e.g., U.S. Pat. No. 3,458,530);

Carbon disulfide (e.g., U.S. Pat. No. 3,256,185);

Glycidol (e.g., U.S. Pat. No. 4,617,137);

Urea, thiourea or guanidine (e.g., U.S. Pat. Nos. 3,312,619; 3,865,813; and British Patent GB 1,065,595);

Organic sulfonic acid (e.g., U.S. Pat. No. 3,189,544 and British Patent GB 2,140,811);

Alkenyl cyanide (e.g., U.S. Pat. Nos. 3,278,550 and 3,366,569);

Diketene (e.g., U.S. Pat. No. 3,546,243);

A diisocyanate (e.g., U.S. Pat. No. 3,573,205);

Alkane sultone (e.g., U.S. Pat. No. 3,749,695);

1,3-Dicarbonyl Compound (e.g., U.S. Pat. No. 4,579,675);

Sulfate of alkoxylated alcohol or phenol (e.g., U.S. Pat. No. 3,954,639);

Cyclic lactone (e.g., U.S. Pat. Nos. 4,617,138; 4,645,515; 4,668,246; 4,963,275; and 4,971,711);

Cyclic carbonate or thiocarbonate linear monocarbonate or polycarbonate, or chloroformate (e.g., U.S. Pat. Nos. 4,612,132; 4,647,390; 4,648,886; 4,670,170);

Nitrogen-containing carboxylic acid (e.g., U.S. Pat. No. 4,971,598 and British Patent GB 2,140,811);

Hydroxy-protected chlorodicarbonyloxy compound (e.g., U.S. Pat. No. 4,614,522);

Lactam, thiolactam, thiolactone or dithiolactone (e.g., U.S. Pat. Nos. 4,614,603 and 4,666,460);

Cyclic carbonate or thiocarbonate, linear monocarbonate or polycarbonate, or chloroformate (e.g., U.S. Pat. Nos. 4,612,132; 4,647,390; 4,646,886; and 4,670,170);

Nitrogen-containing carboxylic acid (e.g., U.S. Pat. No. 4,971,598 and British Patent GB 2,440,811);

Hydroxy-protected chlorodicarbonyloxy compound (e.g., U.S. Pat. No. 4,614,522);

Lactam, thiolactam, thiolactone or dithiolactone (e.g., U.S. Pat. Nos. 4,614,603, and 4,666,460);

Cyclic carbamate, cyclic thiocarbamate or cyclic dithiocarbamate (e.g., U.S. Pat. Nos. 4,663,062 and 4,666,459);

Hydroxyaliphatic carboxylic acid (e.g., U.S. Pat. Nos. 4,482,464; 4,521,318; 4,713,189);

Oxidizing agent (e.g., U.S. Pat. No. 4,379,064);

Combination of phosphorus pentasulfide and a polyalkylene polyamine (e.g., U.S. Pat. No. 3,185,647);

Combination of carboxylic acid or an aldehyde or ketone and sulfur or sulfur chloride (e.g., U.S. Pat. Nos. 3,390,086; 3,470,098);

Combination of a hydrazine and carbon disulfide (e.g. U.S. Pat. No. 3,519,564);

Combination of an aldehyde and a phenol (e.g., U.S. Pat. Nos. 3,649,229; 5,030,249; 5,039,307);

Combination of an aldehyde and an O-diester of dithiophosphoric acid (e.g., U.S. Pat. No. 3,865,740);

Combination of a hydroxyaliphatic carboxylic acid and a boric acid (e.g., U.S. Pat. No. 4,554,086);

## 21

Combination of a hydroxyaliphatic carboxylic acid, then formaldehyde and a phenol (e.g., U.S. Pat. No. 4,636,322);

Combination of a hydroxyaliphatic carboxylic acid and then an aliphatic dicarboxylic acid (e.g., U.S. Pat. No. 4,663,064);

Combination of formaldehyde and a phenol and then glycolic acid (e.g., U.S. Pat. No. 4,699,724);

Combination of a hydroxyaliphatic carboxylic acid or oxalic acid and then a diisocyanate (e.g. U.S. Pat. No. 4,713,191);

Combination of inorganic acid or anhydride of phosphorus or a partial or total sulfur analog thereof and a boron compound (e.g., U.S. Pat. No. 4,857,214);

Combination of an organic diacid then an unsaturated fatty acid and then a nitroaromatic amine optionally followed by a boron compound and then a glycolating agent (e.g., U.S. Pat. No. 4,973,412);

Combination of an aldehyde and a triazole (e.g., U.S. Pat. No. 4,963,278);

Combination of an aldehyde and a triazole then a boron compound (e.g., U.S. Pat. No. 4,981,492);

Combination of cyclic lactone and a boron compound (e.g., U.S. Pat. Nos. 4,963,275 and 4,971,711).

The TBN of a suitable dispersant may be from about 10 to about 65 on an oil-free basis, which is comparable to about 5 to about 30 TBN if measured on a dispersant sample containing about 50% diluent oil.

The dispersant, if present, can be used in an amount sufficient to provide up to about 10 wt. %, based upon the total weight of the lubricating oil composition. Another amount of the dispersant that can be used may be about 0.1 wt. % to about 10 wt. %, or about 1 wt. % to about 9 wt. %, or about 2 wt. % to about 8.5 wt. %, or about 2.75 wt. % to about 6.5 wt. %, based upon the total weight of the lubricating oil composition. In some embodiments, the lubricating oil composition utilizes a mixed dispersant system. A single type or a mixture of two or more types of dispersants in any desired ratio may be used.

If the dispersant contains nitrogen, then the amount of dispersant used in the present lubricating oil compositions may be constrained by the ratio of Ca:N in the lubricating oil composition and/or to the total nitrogen content of the lubricating oil composition.

## Friction Modifiers

The lubricating oil compositions herein also may optionally contain one or more friction modifiers. Suitable friction modifiers may comprise metal containing and metal-free friction modifiers and may include, but are not limited to, imidazolines, amides, amines, succinimides, alkoxyLATED amines, alkoxyLATED ether amines, amine oxides, amidoamines, nitriles, betaines, quaternary amines, imines, amine salts, amino guanadine, alkanolamides, phosphonates, metal-containing compounds, glycerol esters, sulfurized fatty compounds and olefins, sunflower oil other naturally occurring plant or animal oils, dicarboxylic acid esters, esters or partial esters of a polyol and one or more aliphatic or aromatic carboxylic acids, and the like.

Suitable friction modifiers may contain hydrocarbyl groups that are selected from straight chain, branched chain, or aromatic hydrocarbyl groups or mixtures thereof, and may be saturated or unsaturated. The hydrocarbyl groups may be composed of carbon and hydrogen or hetero atoms such as sulfur or oxygen. The hydrocarbyl groups may range from about 12 to about 25 carbon atoms. In some embodiments the friction modifier may be a long chain fatty acid ester. In another embodiment the long chain fatty acid ester

## 22

may be a mono-ester, or a di-ester, or a (tri)glyceride. The friction modifier may be a long chain fatty amide, a long chain fatty ester, a long chain fatty epoxide derivatives, or a long chain imidazoline.

Other suitable friction modifiers may include organic, ashless (metal-free), nitrogen-free organic friction modifiers. Such friction modifiers may include esters formed by reacting carboxylic acids and anhydrides with alkanols and generally include a polar terminal group (e.g. carboxyl or hydroxyl) covalently bonded to an oleophilic hydrocarbon chain. An example of an organic ashless nitrogen-free friction modifier is known generally as glycerol monooleate (GMO) which may contain mono-, di-, and tri-esters of oleic acid. Other suitable friction modifiers are described in U.S. Pat. No. 6,723,685.

Aminic friction modifiers may include amines or polyamines. Such compounds can have hydrocarbyl groups that are linear, either saturated or unsaturated, or a mixture thereof and may contain from about 12 to about 25 carbon atoms. Further examples of suitable friction modifiers include alkoxyLATED amines and alkoxyLATED ether amines. Such compounds may have hydrocarbyl groups that are linear, either saturated, unsaturated, or a mixture thereof. They may contain from about 12 to about 25 carbon atoms. Examples include ethoxyLATED amines and ethoxyLATED ether amines.

The amines and amides may be used as such or in the form of an adduct or reaction product with a boron compound such as a boric oxide, boron halide, metaborate, boric acid or a mono-, di- or tri-alkyl borate. Other suitable friction modifiers are described in U.S. Pat. No. 6,300,291.

A friction modifier may optionally be present in ranges such as about 0 wt. % to about 10 wt. %, or about 0.01 wt. % to about 8 wt. %, or about 0.05 wt. % to about 4 wt. % or about 0.05 to about 2 wt. %, based on the total weight of the lubricating composition.

## Transition Metal-Containing Compounds

In another embodiment, the oil-soluble compound may be a transition metal containing compound or a metalloid. The transition metals may include, but are not limited to, titanium, vanadium, copper, zinc, zirconium, molybdenum, tantalum, tungsten, and the like. Suitable metalloids include, but are not limited to, boron, silicon, antimony, tellurium, and the like.

In one embodiment, the oil-soluble compound that may be used in a weight ratio of Ca/M ranging from about 0.8:1 to about 70:1 is a titanium containing compound, wherein M is the total metal in the lubricant composition as described above. The titanium-containing compounds may function as antiwear agents, friction modifiers, antioxidants, deposit control additives, or more than one of these functions.

Among the titanium containing compounds that may be used in, or which may be used for preparation of the oil-soluble materials of, the disclosed technology are various Ti (IV) compounds such as titanium (IV) oxide; titanium (IV) sulfide; titanium (IV) nitrate; titanium (IV) alkoxides such as titanium methoxide, titanium ethoxide, titanium propoxide, titanium isopropoxide, titanium butoxide, titanium 2-ethylhexoxide; and other titanium compounds or complexes including but not limited to titanium phenates; titanium carboxylates such as titanium (IV) 2-ethyl-1-3-hexanedioate or titanium citrate or titanium oleate; and titanium (IV) (triethanolaminato)isopropoxide. The mono-hydric alkoxides may have 2 to 16, or 3 to 10 carbon atoms.

In an embodiment, the titanium compound may be the alkoxide of a 1,2-diol or polyol. In an embodiment, the 1,2-diol comprises a fatty acid mono-ester of glycerol, such as oleic acid. In an embodiment, the oil soluble titanium compound may be a titanium carboxylate. In an embodiment the titanium (IV) carboxylate may be titanium neodecanoate.

Other forms of titanium encompassed within the disclosed technology include titanium phosphates such as titanium dithiophosphates (e.g., dialkyldithiophosphates) and titanium sulfonates (e.g., alkylbenzenesulfonates), or, generally, the reaction product of titanium compounds with various acid materials to form salts, such as oil-soluble salts. Titanium compounds can thus be derived from, among others, organic acids, alcohols, and glycols. Ti compounds may also exist in dimeric or oligomeric form, containing Ti—O—Ti structures. Such titanium materials are commercially available or can be readily prepared by appropriate synthesis techniques which will be apparent to the person skilled in the art. They may exist at room temperature as a solid or a liquid, depending on the particular compound. They may also be provided in a solution form in an appropriate inert solvent.

In one embodiment, the titanium can be supplied as a Ti-modified dispersant, such as a succinimide dispersant. Such materials may be prepared by forming a titanium mixed anhydride between a titanium alkoxide and a hydrocarbyl-substituted succinic anhydride, such as an alkenyl-(or alkyl) succinic anhydride. The resulting titanate-succinate intermediate may be used directly or it may be reacted with any of a number of materials, such as (a) a polyamine-based succinimide/amide dispersant having free, condensable —NH functionality; (b) the components of a polyamine-based succinimide/amide dispersant, i.e., an alkenyl-(or alkyl-) succinic anhydride and a polyamine, (c) a hydroxy-containing polyester dispersant prepared by the reaction of a substituted succinic anhydride with a polyol, aminoalcohol, polyamine, or mixtures thereof. Alternatively, the titanate-succinate intermediate may be reacted with other agents such as alcohols, aminoalcohols, ether alcohols, polyether alcohols or polyols, or fatty acids, and the product thereof either used directly to impart Ti to a lubricant, or else further reacted with the succinic dispersants as described above. As an example, 1 part (by mole) of tetraisopropyl titanate may be reacted with about 2 parts (by mole) of a polyisobutene-substituted succinic anhydride at 140-150° C. for 5 to 6 hours to provide a titanium modified dispersant or intermediate. The resulting material (30 g) may be further reacted with a succinimide dispersant from polyisobutene-substituted succinic anhydride and a polyethylenepolyamine mixture (127 grams+diluent oil) at 150° C. for 1.5 hours, to produce a titanium-modified succinimide dispersant.

Another titanium containing compound may be a reaction product of titanium alkoxide and C<sub>6</sub> to C<sub>25</sub> carboxylic acid. The reaction product may be represented by the following formula:



wherein n is an integer selected from 2, 3 and 4, and R is a hydrocarbyl group containing from about 5 to about 24 carbon atoms, or by the formula:



wherein  $m+n=4$  and  $n$  ranges from 1 to 3,  $R_4$  is an alkyl moiety with carbon atoms ranging from 1-8,  $R_1$  is selected from a hydrocarbyl group containing from about 6 to 25 carbon atoms, and  $R_2$  and  $R_3$  are the same or different and are selected from a hydrocarbyl group containing from about 1 to 6 carbon atoms, or by the formula:



35 wherein x ranges from 0 to 3, R<sub>1</sub> is selected from a hydrocarbyl group containing from about 6 to 25 carbon atoms, R<sub>2</sub>, and R<sub>3</sub> are the same or different and are selected from a hydrocarbyl group containing from about 1 to 6 carbon atoms, and R<sub>4</sub> is selected from a group consisting of  
40 either H, or C<sub>6</sub> to C<sub>25</sub> carboxylic acid moiety.

Suitable carboxylic acids may include, but are not limited to caproic acid, caprylic acid, lauric acid, myristic acid, palmitic acid, stearic acid, arachidic acid, oleic acid, erucic acid, linoleic acid, linolenic acid, cyclohexanecarboxylic acid, phenylacetic acid, benzoic acid, neodecanoic acid, and the like.

In an embodiment the oil soluble titanium compound may be present in the lubricating oil composition in an amount to provide from 0 to 3000 ppm titanium or 25 to about 1500 ppm titanium or about 35 ppm to 500 ppm titanium or about 50 ppm to about 300 ppm titanium, based on the total weight of the lubricating composition.

## Viscosity Index Improvers

The lubricating oil compositions herein also may optionally contain one or more viscosity index improvers. Suitable viscosity index improvers may include polyolefins, olefin copolymers, ethylene/propylene copolymers, polyisobutenes, hydrogenated styrene-isoprene polymers, styrene/maleic ester copolymers, hydrogenated styrene/butadiene copolymers, hydrogenated isoprene polymers, alpha-olefin maleic anhydride copolymers, polymethacrylates, polyacrylates, polyalkyl styrenes, hydrogenated alkaryl conjugated diene copolymers, or mixtures thereof. Viscosity index improvers may include star polymers and suitable examples are described in U.S. Pat. No. 8,999,905 B2.

The lubricating oil compositions herein also may optionally contain one or more dispersant viscosity index improvers.

ers in addition to a viscosity index improver or in lieu of a viscosity index improver. Suitable viscosity index improvers may include functionalized polyolefins, for example, ethylene-propylene copolymers that have been functionalized with the reaction product of an acylating agent (such as maleic anhydride) and an amine; polymethacrylates functionalized with an amine, or esterified maleic anhydride-styrene copolymers reacted with an amine.

The total amount of viscosity index improver and/or dispersant viscosity index improver may be about 0 wt. % to about 20 wt. %, about 0.1 wt. % to about 15 wt. %, about 0.1 wt. % to about 12 wt. %, or about 0.25 wt. % to about 11 wt. %, or about 3 to about 10.5 wt. %, based on a total weight of the lubricating oil composition.

#### Other Optional Additives

Other additives may be selected to perform one or more functions required of a lubricating fluid. Further, one or more of the mentioned additives may be multi-functional and provide functions in addition to or other than the function prescribed herein.

A lubricating oil composition according to the present disclosure may optionally comprise other performance additives. The other performance additives may be in addition to specified additives of the present disclosure and/or may comprise one or more of metal deactivators, viscosity index improvers, ashless TBN boosters, friction modifiers, anti-wear agents, corrosion inhibitors, rust inhibitors, dispersants, dispersant viscosity index improvers, extreme pressure agents, antioxidants, foam inhibitors, demulsifiers, emulsifiers, pour point depressants, seal swelling agents and mixtures thereof. Typically, fully-formulated lubricating oil will contain one or more of these performance additives.

Suitable metal deactivators may include derivatives of benzotriazoles (typically tolyltriazole), dimercaptothiadiazole derivatives, 1,2,4-triazoles, benzimidazoles, 2-alkyldithiobenzimidazoles, or 2-alkyldithiobenzothiazoles; foam inhibitors including copolymers of ethyl acrylate and 2-ethylhexylacrylate and optionally vinyl acetate; demulsifiers including trialkyl phosphates, polyethylene glycols, poly-ethylene oxides, polypropylene oxides and (ethylene oxide-propylene oxide) polymers; pour point depressants including esters of maleic anhydride-styrene, polymethacrylates, polyacrylates or polyacrylamides.

Suitable foam inhibitors include silicon-based compounds, such as siloxane.

Suitable pour point depressants may include a polymethylmethacrylates or mixtures thereof. Pour point depressants may be present in an amount sufficient to provide from about 0 wt. % to about 5 wt. %, about 0.01 wt. % to about 3 wt. %, or about 0.01 wt. % to about 1.5 wt. % based upon the total weight of the lubricating oil composition.

Suitable rust inhibitors may be a single compound or a mixture of compounds having the property of inhibiting corrosion of ferrous metal surfaces. Non-limiting examples of rust inhibitors useful herein include oil-soluble high molecular weight organic acids, such as 2-ethylhexanoic acid, lauric acid, myristic acid, palmitic acid, oleic acid, linoleic acid, linolenic acid, behenic acid, and cerotic acid, as well as oil-soluble polycarboxylic acids including dimer and trimer acids, such as those produced from tall oil fatty acids, oleic acid, and linoleic acid. Other suitable corrosion inhibitors include long-chain alpha, omega-dicarboxylic acids in the molecular weight range of about 600 to about 3000 and alkenylsuccinic acids in which the alkenyl group contains about 10 or more carbon atoms such as, tetrapropenylsuccinic acid, tetradecenylsuccinic acid, and hexadecenylsuccinic acid. Another useful type of acidic corrosion

inhibitors are the half esters of alkenyl succinic acids having about 8 to about 24 carbon atoms in the alkenyl group with alcohols such as the polyglycols. The corresponding half amides of such alkenyl succinic acids are also useful. A useful rust inhibitor is a high molecular weight organic acid. In some embodiments, an engine oil is devoid of a rust inhibitor.

The rust inhibitor, if present, can be used in an amount sufficient to provide about 0 wt. % to about 5 wt. %, about 0.01 wt. % to about 3 wt. %, about 0.1 wt. % to about 2 wt. %, based upon the total weight of the lubricating oil composition.

In general terms, a suitable crankcase lubricant may include additive components in the ranges listed in the following table.

TABLE 2

| Component                              | Wt. %<br>(Broad) | Wt. %<br>(Typical) |
|----------------------------------------|------------------|--------------------|
| Dispersant(s)                          | 0.0-10%          | 1.0-8.5%           |
| Antioxidant(s)                         | 0.0-5.0          | 0.01-3.0           |
| Metal Detergent(s)                     | 0.1-15.0         | 0.2-8.0            |
| Ashless TBN booster(s)                 | 0.0-1.0          | 0.01-0.5           |
| Corrosion Inhibitor(s)                 | 0.0-5.0          | 0.0-2.0            |
| Metal dihydrocarbyl dithiophosphate(s) | 0.1-6.0          | 0.1-4.0            |
| Ash-free amine phosphate salt(s)       | 0.0-3.0          | 0.0-1.5            |
| Antifoaming agent(s)                   | 0.0-5.0          | 0.001-0.15         |
| Antiwear agent(s)                      | 0.0-10.0         | 0.0-5.0            |
| Pour point depressant(s)               | 0.0-5.0          | 0.01-1.5           |
| Viscosity index improver(s)            | 0.0-20.00        | 0.25-11.0          |
| Dispersant viscosity index improver(s) | 0.0-10.0         | 0.0-5.0            |
| Friction modifier(s)                   | 0.0-5.0          | 0.05-2.0           |
| Base oil(s)                            | Balance          | Balance            |
| Total                                  | 100              | 100                |

The percentages of each component above represent the weight percent of each component, based upon the total weight of the lubricating oil composition. The remainder of the lubricating oil composition consists of one or more base oils.

Additives used in formulating the compositions described herein may be blended into the base oil individually or in various sub-combinations. However, it may be suitable to blend all of the components concurrently using an additive concentrate (i.e., additives plus a diluent, such as a hydrocarbon solvent). Additives used in formulating the compositions described herein may be blended into the base oil individually or in various sub-combinations. However, it may be suitable to blend all of the components concurrently using an additive concentrate (i.e., additives plus a diluent, such as a hydrocarbon solvent).

The present disclosure provides novel lubricating oil blends specifically formulated for use as automotive engine lubricants. Embodiments of the present disclosure may provide lubricating oils suitable for engine applications that provide improvements in one or more of the following characteristics: antioxidant, antiwear performance, rust inhibition, fuel economy, water tolerance, air entrainment, seal protection, and turbocharger deposit reduction, i.e., resisting TCO Temperature Increase.

Fully formulated lubricants conventionally contain an additive package, referred to herein as a dispersant/inhibitor package or DI package, that will supply the characteristics that are required in the formulations. Suitable DI packages are described for example in U.S. Pat. Nos. 5,204,012 and 6,034,040 for example. Among the types of additives included in the additive package may be dispersants, seal

swell agents, antioxidants, foam inhibitors, lubricity agents, rust inhibitors, corrosion inhibitors, demulsifiers, viscosity index improvers, and the like. Several of these components are well known to those skilled in the art and are generally used in conventional amounts with the additives and compositions described herein.

The following examples are illustrative, but not limiting, of the methods and compositions of the present disclosure. Other suitable modifications and adaptations of the variety of conditions and parameters normally encountered in the field, and which are obvious to those skilled in the art, are within the scope of the disclosure.

### EXAMPLES

Fully formulated lubricating oil compositions containing additives were made and tested to determine their influence on turbocharger deposit formation by testing the resistance to TCO Temperature Increase in a boosted internal combustion engine. The TCO Temperature Increase provides an indication that deposits in the engine are producing an insulating effect. Thus, an increase in the TCO Temperature of a turbocharger of a boosted internal combustion engine indicates an increase in the amount of turbocharger deposits.

Each of the lubricating oil compositions contained a major amount of a base oil, a DI package and one or more viscosity index improver(s), wherein the DI package (less the viscosity index improver) provided about 8 to about 16 percent by weight of the lubricating oil composition. The DI package contained conventional amounts of dispersant(s), antiwear additive(s), antifoam agent(s), and antioxidant(s) as set forth in Table 3 below. Specifically, the DI package contained a succinimide dispersant, a borated succinimide dispersant, a molybdenum-containing compound, a friction modifier, one or more antioxidants, and one or more anti-wear agents (unless specified otherwise). About 4 to about 10 wt. % of one or more viscosity index improver(s) was included in each tested lubricating oil composition. A base oil was used as a diluent oil for the viscosity index improver(s). The components that were varied are specified in the Tables and discussion of the Examples given below. All the values listed in Table 3 are stated as weight percent of the component based on the total weight of the lubricating oil composition (i.e., active ingredient plus diluent oil, if any), unless specified otherwise.

TABLE 3

| DI Package Composition Ranges                                        |               |
|----------------------------------------------------------------------|---------------|
| Component                                                            | Wt. %         |
| Antioxidant(s)                                                       | 0.4 to 2.8    |
| Antiwear agent(s), including any metal dihydrocarbyl dithiophosphate | 0.7 to 5.0    |
| Antifoaming agent(s)                                                 | 0.001 to 0.01 |
| Detergent(s)                                                         | 0.5 to 5.0    |
| Dispersant(s)                                                        | 2.0 to 8.0    |
| Metal-containing friction modifier(s)                                | 0.0 to 1.25   |
| Metal free friction modifier(s)                                      | 0.01 to 1.0   |
| Pour point depressant(s)                                             | 0.05 to 0.5   |
| Process oil                                                          | 0.25 to 1.0   |

#### Turbocharger Coking Test

The turbocharger coking tests were carried out using a 2012, 1.4 L Chevy Cruze calibration engine with 3 liters of test oil charge and a qualified test fuel using the 2015 version of the General Motors dexos1® Turbocharger Coking Test (TC Test).

The TCO Temperature is measured every 30 seconds. The “100 cycle TCO Temperature” is the average TCO temperature of cycle 1 to cycle 100 of the TC test. The “1800 cycle TCO Temperature” is the average TCO temperature from cycle 1701 to cycle 1800 of the TC Test. The test is considered a “pass” if the TCO Temperature Increase from the 100 cycle TCO Temperature to the 1800 cycle TCO Temperature is less than 9.0%.

<sup>10</sup> Comparative Examples C-1 and C-2 and Inventive Examples I-1, I-2 and I-3

<sup>15</sup> In the following examples, the impact of the incorporation of calcium, nitrogen, molybdenum and boron in varying ratios on the TCO Temperature Increase was determined. The amounts of calcium, nitrogen, molybdenum, boron and magnesium were determined by ICP analysis.

<sup>20</sup> Five samples were tested, each containing greater than 50 wt. % of a base oil of lubricating viscosity; and the elements of calcium, nitrogen, molybdenum and boron, and none containing added magnesium from a magnesium-containing detergent.

TABLE 4

|                                                          | Components |        |            |        |        |
|----------------------------------------------------------|------------|--------|------------|--------|--------|
|                                                          | Base Oil   |        | Components |        |        |
|                                                          | C-1        | C-2    | I-1        | I-2    | I-3    |
| <sup>30</sup>                                            | II/III     | III    | III        | III    | III    |
| Weight Ratio of Total Calcium:Total Nitrogen (ppm/ppm)   | 3.0        | 1.3    | 2.1        | 1.8    | 1.6    |
| <sup>35</sup>                                            | 56.3       | 6.7    | 29.1       | 6.9    | 20.0   |
| Weight Ratio of Total Calcium:Total Molybdenum (ppm/ppm) | 9.8        | 4.3    | 6.0        | 7.1    | 5.4    |
| <sup>40</sup>                                            | No         | No     | No         | No     | No     |
| Weight Ratio of Total Calcium:Total Boron (ppm/ppm)      | 21.1       | 9.2    | 4.2        | 4.2    | 0.8    |
| <sup>45</sup>                                            | (Fail)     | (Fail) | (Pass)     | (Pass) | (Pass) |
| Mg from Mg Detergent present? (Yes/No)                   |            |        |            |        |        |
| TCO Temperature Increase (%) <sup>a</sup>                |            |        |            |        |        |

<sup>50</sup> <sup>a</sup>Percent increase in TCO Temperature. “Pass” means that the TCO Temperature Increase was less than 9.0%.

<sup>55</sup> Comparative examples C-1 and C-2 are not commercially available fluids but instead are fluids designed to demonstrate technical problems experienced by one skilled in the art when the lubricant oil composition is modified to meet performance needs.

In Table 4, formulations C-1, C-2, I-1, I-2 and I-3 demonstrate the relationship between the calcium:nitrogen weight ratio and the TCO Temperature Increase. When the calcium:nitrogen weight ratio is outside the range of greater than 1.3 to less than 3.0, as in Comparative examples C-1 and C-2, the lubricating oil composition failed the TC test since the TCO Temperature Increase was 9.0% or greater. On the other hand, each of the lubricating oil compositions of Inventive examples I-1, I-2 and I-3 having a calcium:nitrogen weight ratio which is inside the range of greater than 1.3 to less than 3.0, passed the TC test, i.e., the TCO

Temperature Increase was less than 9.0%. Accordingly, Inventive examples I-1, I-2 and I-3 showed an improved resistance to formation of turbocharger deposits in a boosted engine.

In Table 4, formulations C-1, C-2, I-1, I-2 and I-3 demonstrate the relationship between the calcium:molybdenum weight ratio and the TCO Temperature Increase. When the calcium:molybdenum weight ratio is outside the range of greater than 6.7 to less than 56.3, as in Comparative examples C-1 and C-2, the lubricating oil composition failed the TC test since the TCO Temperature Increase was 9.0% or greater. On the other hand, each of the lubricating oil compositions of Inventive examples I-1, I-2 and I-3 having a calcium:molybdenum weight ratio which is inside the range of greater than 6.7 to less than 56.3, passed the TC test, i.e., the TCO Temperature Increase was less than 9.0%. Accordingly, Inventive examples I-1, I-2 and I-3 showed an improved resistance to formation of turbocharger deposits in a boosted engine.

In Table 4, formulations C-1, C-2, I-1, I-2 and I-3 demonstrate the relationship between the calcium:boron weight ratio and the TCO Temperature Increase. When the calcium:boron weight ratio is outside the range of greater than 5.0 to less than 9.8, as in Comparative examples C1 and C-2, the lubricating oil composition failed the TC test since the TCO Temperature Increase was 9.0%. On the other hand, each of the lubricating oil compositions of Inventive examples I-1, I-2 and I-3 having a calcium:boron weight ratio which is inside the range of greater than 5.0 to less than 9.8, passed the TC test, i.e., the TCO Temperature Increase was less than 9.0%. Accordingly, Inventive examples I-1, I-2 and I-3 showed an improved resistance to formation of turbocharger deposits in a boosted engine.

At numerous places throughout this specification, reference has been made to a number of U.S. Patents and other documents. All such cited documents are expressly incorporated in full into this disclosure as if fully set forth herein and/or for the purpose that they are cited in the text.

Other embodiments of the present disclosure will be apparent to those skilled in the art from consideration of the specification and practice of the embodiments disclosed herein. As used throughout the specification and claims, "a" and/or "an" may refer to one or more than one. Unless otherwise indicated, all numbers expressing quantities of ingredients, properties such as molecular weight, percent, ratio, reaction conditions, and so forth used in the specification and claims are to be understood as being modified in all instances by the term "about," whether or not the term "about" is present. Accordingly, unless indicated to the contrary, the numerical parameters set forth in the specification and claims are approximations that may vary depending upon the desired properties sought to be obtained by the present disclosure. At the very least, and not as an attempt to limit the application of the doctrine of equivalents to the scope of the claims, each numerical parameter should at least be construed in light of the number of reported significant digits and by applying ordinary rounding techniques. Notwithstanding that the numerical ranges and parameters setting forth the broad scope of the disclosure are approximations, the numerical values set forth in the specific examples are reported as precisely as possible. Any numerical value, however, inherently contains certain errors necessarily resulting from the standard deviation found in their respective testing measurements. It is intended that the specification and examples be considered as exemplary only, with a true scope of the disclosure being indicated by the following claims.

The foregoing embodiments are susceptible to considerable variation in practice. Accordingly, the embodiments are not intended to be limited to the specific exemplifications set forth hereinabove. Rather, the foregoing embodiments are within the scope of the appended claims, including the equivalents thereof available as a matter of law.

The patentees do not intend to dedicate any disclosed embodiments to the public, and to the extent any disclosed modifications or alterations may not literally fall within the scope of the claims, they are considered to be part hereof under the doctrine of equivalents.

It is to be understood that each component, compound, substituent or parameter disclosed herein is to be interpreted as being disclosed for use alone or in combination with one or more of each and every other component, compound, substituent or parameter disclosed herein.

It is also to be understood that each amount/value or range of amounts/values for each component, compound, substituent or parameter disclosed herein is to be interpreted as also being disclosed in combination with each amount/value or range of amounts/values disclosed for any other component(s), compounds(s), substituent(s) or parameter(s) disclosed herein and that any combination of amounts/values or ranges of amounts/values for two or more component(s), compounds(s), substituent(s) or parameters disclosed herein are thus also disclosed in combination with each other for the purposes of this description.

It is further understood that each range disclosed herein is to be interpreted as a disclosure of each specific value within the disclosed range that has the same number of significant digits. Thus, a range of from 1-4 is to be interpreted as an express disclosure of the values 1, 2, 3 and 4.

It is further understood that each lower limit of each range disclosed herein is to be interpreted as disclosed in combination with each upper limit of each range and each specific value within each range disclosed herein for the same component, compounds, substituent or parameter. Thus, this disclosure to be interpreted as a disclosure of all ranges derived by combining each lower limit of each range with each upper limit of each range or with each specific value within each range, or by combining each upper limit of each range with each specific value within each range.

Furthermore, specific amounts/values of a component, compound, substituent or parameter disclosed in the description or an example is to be interpreted as a disclosure of either a lower or an upper limit of a range and thus can be combined with any other lower or upper limit of a range or specific amount/value for the same component, compound, substituent or parameter disclosed elsewhere in the application to form a range for that component, compound, substituent or parameter.

What is claimed is:

1. A method for reducing or preventing formation of deposits in a boosted internal combustion engine comprising steps of:

lubricating a boosted internal combustion engine with a lubricating oil composition comprising  
greater than 50 wt. % of a base oil of lubricating  
viscosity;  
a boron-containing dispersant,  
an oil-soluble molybdenum compound present in an  
amount to provide 0.5 ppm to about 2,000 ppm by  
weight of molybdenum to the lubricating oil com-  
position,  
wherein the lubricating oil composition comprises cal-  
cium, nitrogen, molybdenum and boron,

31

a weight ratio of Ca:N in the lubricating oil composition is 1.4 to less than 2.3, a weight ratio of Ca:Mo in the lubricating oil composition is greater than 6.7 to less than 56.3, a weight ratio of Ca:B in the lubricating oil composition is greater than 5.0 to less than 9.8, wherein the lubricating oil composition comprises at least one detergent selected from one or more overbased calcium-containing detergents having a total base number of greater than 225 mg KOH/g, measured by the method of ASTM D-2896 in an amount that provides from 900 to 3,000 ppm by weight calcium to the lubricating oil composition, based on a total weight of the lubricating oil composition, and wherein the nitrogen is present in the lubricating oil composition in an amount of from 500 ppm to 2,500 ppm, based on a total weight of the lubricating oil composition, and

the lubricating oil composition does not contain added magnesium from a magnesium-containing detergent and the lubricating oil composition contains less than 100 ppm of sodium, and

the lubricating oil composition is effective to ensure a TCO Temperature Increase of less than 9.0% as measured using the 2015 version of the General Motors dexos1® Turbocharger Coking Test, and operating the engine lubricated with the lubricating oil composition.

2. The method of claim 1, wherein the lubricating oil composition comprises one or more low-based/neutral calcium-containing detergents having a total base number of up to 175 mg KOH/g, measured by the method of ASTM D-2896.

3. The method of claim 2, wherein the one or more overbased calcium-containing detergents provides from 1,300 to 2,500 ppm by weight calcium to the lubricating oil composition, based on a total weight of the lubricating oil composition.

4. The method of claim 2, wherein the one or more overbased calcium-containing detergents is selected from an overbased calcium sulfonate detergent, an overbased calcium phenate detergent, an overbased calcium salicylate detergent and mixtures thereof.

5. The method of claim 1, wherein the nitrogen is present in the lubricating oil composition in an amount of from about 900 ppm to about 1,600 ppm, based on a total weight of the lubricating oil composition.

6. The method of claim 1, wherein the lubricating step lubricates a combustion chamber or cylinder walls of a spark-ignited direct injection engine or spark-ignited port fuel injected internal combustion engine provided with a turbocharger or a supercharger.

7. The method of claim 1, wherein the total base number of the lubricating oil composition is at least 6.0 mg KOH/g of the lubricating oil composition as measured by the method of ASTM D-2896.

32

8. The method according to claim 1, wherein the total amount of magnesium in the lubricating oil composition is less than 50 ppm, based on a total weight of the lubricating oil composition and the lubricating oil composition contains 50 ppm or less of sodium.

9. The method of claim 1, further comprising one or more components selected from the group consisting of friction modifiers, antiwear agents, dispersants, antioxidants, and viscosity index improvers.

10. The method of claim 9, wherein the lubricant composition comprises 4 to less than 10 wt. % of the viscosity index improver, and the viscosity index improver is not a dispersant viscosity index improver.

11. The method of claim 10, wherein the viscosity index improver is selected from the group consisting of polyolefins, olefin copolymers, ethylene/propylene copolymers, polyisobutene, hydrogenated styrene-isoprene polymers, hydrogenated styrene/butadiene copolymers, hydrogenated isoprene polymers, polyalkyl styrenes, hydrogenated alk-20 enyl aryl conjugated diene copolymers, and mixtures thereof.

12. The method of claim 1, wherein the greater than 50 wt. % of base oil is selected from the group consisting of Group II, Group III, Group IV, Group V base oils, and a combination of two or more of the foregoing, and wherein the greater than 50 wt. % of base oil is other than diluent oils that arise from provision of additive components or viscosity index improvers in the composition.

13. The method of claim 1, wherein the weight ratio of Ca:N in the lubricating oil composition is from 1.4 to 2.1.

14. The method of claim 1, wherein the weight ratio of Ca:Mo in the lubricating oil composition is from 6.8 to 45.

15. The method of claim 1, wherein the weight ratio of Ca:B in the lubricating oil composition is from greater than 5.1 to 9.7.

16. The method of claim 1, wherein the lubricating oil composition is effective to ensure a TCO Temperature Increase of less than 8.0% as measured using the 2015 version of the General Motors dexos1® Turbocharger Coking Test.

17. The method of claim 1, wherein the weight ratio of Ca:N in the lubricating oil composition is from 1.4 to 2.1, the weight ratio of Ca:Mo in the lubricating oil composition is from 6.8 to 45, and the weight ratio of Ca:B in the lubricating oil composition is from greater than 5.1 to 9.7.

18. The method of claim 1, wherein the weight ratio of Ca:N in the lubricating oil composition is from 1.6 to 2.1, the weight ratio of Ca:Mo in the lubricating oil composition is from 6.9 to 29.1, and the weight ratio of Ca:B in the lubricating oil composition is from 5.4 to 7.1.

19. The method of claim 1, wherein the oil-soluble molybdenum compound is present in an amount to provide 5 ppm to about 300 ppm by weight of molybdenum to the lubricating oil composition.

\* \* \* \* \*